



US007906267B2

(12) **United States Patent**  
Shinohara et al.

(10) **Patent No.:** US 7,906,267 B2  
(45) **Date of Patent:** Mar. 15, 2011

(54) **HEAT-SENSITIVE TRANSFER  
IMAGE-RECEIVING SHEET**

(75) Inventors: **Ryuji Shinohara**, Minami-ashigara (JP);  
**Toshihide Yoshitani**, Minami-ashigara (JP)

(73) Assignee: **FUJIFILM Corporation**, Tokyo (JP)

(\*) Notice: Subject to any disclaimer, the term of this patent is extended or adjusted under 35 U.S.C. 154(b) by 0 days.

(21) Appl. No.: **11/878,818**

(22) Filed: **Jul. 27, 2007**

(65) **Prior Publication Data**

US 2008/0026323 A1 Jan. 31, 2008

(30) **Foreign Application Priority Data**

Jul. 28, 2006 (JP) ..... 2006-206500

(51) **Int. Cl.**

**G03C 8/00** (2006.01)

**B41M 5/40** (2006.01)

**B41M 5/20** (2006.01)

**B41M 5/24** (2006.01)

(52) **U.S. Cl.** .... **430/201**; 503/227; 428/32.6; 428/32.39;  
428/32.85; 428/32.86

(58) **Field of Classification Search** ..... 430/201;  
428/32.85, 32.39, 32.6, 32.86, 32.64; 503/227  
See application file for complete search history.

(56) **References Cited**

U.S. PATENT DOCUMENTS

3,635,719 A \* 1/1972 Ohkubo et al. ..... 430/350  
4,140,532 A \* 2/1979 Sato et al. ..... 430/495.1

4,281,060 A \* 7/1981 Usami et al. ..... 430/618  
5,071,823 A \* 12/1991 Matsushita et al. ..... 503/227  
5,358,922 A \* 10/1994 Nakayama et al. ..... 503/227  
5,372,987 A \* 12/1994 Fisch et al. ..... 503/227  
5,418,057 A \* 5/1995 Tokiyoshi et al. ..... 428/32.39  
5,582,941 A \* 12/1996 Kato et al. ..... 430/47.3  
5,643,709 A \* 7/1997 Kamio et al. ..... 430/201  
5,902,770 A \* 5/1999 Narita et al. ..... 503/227  
5,916,842 A \* 6/1999 Morimitsu et al. ..... 503/227  
6,372,689 B1 \* 4/2002 Kuga et al. ..... 503/227  
6,692,879 B2 \* 2/2004 Suzuki et al. ..... 430/17  
7,223,513 B2 5/2007 Nakane et al. ..... 428/32.39  
2005/0266185 A1 \* 12/2005 Sekiya et al. ..... 428/32.39

FOREIGN PATENT DOCUMENTS

|    |              |         |
|----|--------------|---------|
| JP | 4-284292 A   | 10/1992 |
| JP | 5-8572       | 1/1993  |
| JP | 6-171240 A   | 6/1994  |
| JP | 7-17148 A    | 1/1995  |
| JP | 2541796      | 7/1996  |
| JP | 2726040      | 12/1997 |
| JP | 11-58993 A   | 3/1999  |
| JP | 11-227345 A  | 8/1999  |
| JP | 3226167      | 8/2001  |
| JP | 2006-88691   | 4/2006  |
| JP | 2006-88691 A | 4/2006  |

\* cited by examiner

*Primary Examiner* — Amanda C. Walke

(74) *Attorney, Agent, or Firm* — Sughrue Mion, PLLC

(57) **ABSTRACT**

A heat-sensitive transfer image-receiving sheet, containing; a support; at least one receptor layer containing at least two kinds of latex polymers, said latex polymers having different elastic moduli from each other; and at least one heat-insulation layer containing hollow latex polymer particles and a water-soluble polymer, said at least one heat-insulation layer being provided between the support and the at least one receptor layer.

**21 Claims, No Drawings**

## 1

HEAT-SENSITIVE TRANSFER  
IMAGE-RECEIVING SHEET

## FIELD OF THE INVENTION

The present invention relates to a heat-sensitive transfer image-receiving sheet.

## BACKGROUND OF THE INVENTION

Various heat transfer recording methods have been known so far. Among these methods, dye diffusion transfer recording systems attract attention as a process that can produce a color hard copy having an image quality closest to that of silver halide photography (see, for example, "Joho Kiroku (Hard Copy) to Sono Zairyō no Shintenkai (Information Recording (Hard Copy) and New Development of Recording Materials)" published by Toray Research Center Inc., 1993, pp. 241-285; and "Printer Zairyō no Kaihatsu (Development of Printer Materials)" published by CMC Publishing Co., Ltd., 1995, p. 180). Moreover, this system has advantages over silver halide photography: it is a dry system, it enables direct visualization from digital data, it makes reproduction simple, and the like.

In this dye diffusion transfer recording system, a heat-sensitive transfer sheet (hereinafter also referred to as an ink sheet) containing dyes is superposed on a heat-sensitive transfer image-receiving sheet (hereinafter also referred to as an image-receiving sheet), and then the ink sheet is heated by a thermal head whose exothermic action is controlled by electric signals, in order to transfer the dyes contained in the ink sheet to the image-receiving sheet, thereby recording an image information. Three colors: cyan, magenta, and yellow, are used for recording a color image by overlapping one color to other, thereby enabling transferring and recording a color image having continuous gradation for color densities.

In such a recording method in dye diffusion transfer system, it has been known that it is important to make the image-receiving sheet have high heat insulation and cushion characteristics in order to give a favorable image (see, for example, "Joho Kiroku (Hard Copy) to Sono Zairyō no Shintenkai (Information Recording (Hard Copy) and New Development of Recording Materials)" published by Toray Research Center Inc., 1993, pp. 241-285 and "Printer Zairyō no Kaihatsu (Development of Printer Materials)" published by CMC Publishing Co., Ltd., 1995, p. 180).

Thus, in some cases, a composite support using a biaxial oriented (stretched) polyolefin film containing microvoids was used as a base material for the image-receiving sheet to make the sheet have more heat insulation and cushion characteristics (see, for example, U.S. Pat. No. 866,282 and JP-A-3-268998 ("JP-A" means unexamined published Japanese patent application)). However in this method, there was occasionally caused a problem that the image-receiving sheet was wrinkled or curled by shrinkage due to relaxation of the residual stress after stretching by the heat during printing or the heat during formation of the image-receiving layer.

As other known methods of making the image-receiving sheet show heat insulation and cushion characteristics, a method in which, for example, a foaming layer composed of a resin and a foaming agent (see, e.g., Japanese Patent No. 2541796) or a porous layer containing hollow polymer particles (see, e.g., Japanese Patent No. 2726040) each having high cushion characteristics is formed between the support and the receptor layer, is known. The methods have an advantage that it is possible to prevent the image-receiving sheet from wrinkling and curling that are often found in the method

## 2

in which a composite support made of a biaxially-oriented polyolefin film containing microvoids is used, because a heat-insulating layer can be formed on a base material by coating according to the method. However, it is generally difficult to produce a uniform smooth image-receiving sheet often causing problems such as poor image-transfer or transfer failure owing to insufficient contact between the ink sheet and the image-receiving sheet.

To solve the problems described above, an image-receiving sheet having a heat insulation layer made of hollow polymer particles and an organic solvent-resistant polymer as principal components is disclosed (see, e.g., Japanese Patent No. 3226167). However, the image-receiving sheet has not met a sufficient level. In addition, a method in which a solution for forming an intermediate layer is coated on a sheet-shaped base material and an image-receiving sheet is formed while pressing the coated face to a cast drum in forming an intermediate layer of a resin containing hollow particles as the principal component on the sheet-shaped base material, is disclosed (see, e.g., JP-A-5-8572). However, although such a method is effective in giving sufficient smoothness, it makes the production process more complicated and is thus disadvantageous from the viewpoint of productivity.

On the other hand, it is known, in the field of silver salt photography, that productivity can be greatly improved by simultaneously providing plural layers which have functions different from each other on a support through multi-layer coating of using aqueous coating solutions (see, for example, JP-A-63-54975 and Edgar B. Gutoff, et al., "Coating and Drying Defects: Troubleshooting Operating Problems", John Wiley & Sons Company, 1995, pp. 101-103).

There is known a method of producing an image-receiving sheet using such the multilayer coating of using aqueous coating solutions (see, for example, JP-A-2006-88691). However, it is difficult to achieve sufficient cushion characteristics according to the method. Consequently, it causes transfer failure owing to insufficient contact between the ink sheet and the image-receiving sheet. This is because hollow polymer particles are so hard that it is difficult to achieve sufficient cushion characteristics, compared to the above-described "composite support made of a biaxially-oriented polyolefin film containing microvoids".

It has been desired to improve a heat-sensitive transfer image-receiving sheet so that it causes no transfer failure and exhibits high cushion characteristics, and also to improve a method of producing the heat-sensitive transfer image-receiving sheet, by applying the multilayer coating technology using aqueous coating solutions that is preferable from technical viewpoints such as air pollution, fire hazard, sanitary working conditions as well as productivity, compared to the organic solvent based coating.

## SUMMARY OF THE INVENTION

The present invention resides in a heat-sensitive transfer image-receiving sheet, comprising;

a support;  
at least one receptor layer containing at least two kinds of latex polymers, said latex polymers having different elastic moduli from each other; and

at least one heat-insulation layer containing hollow latex polymer particles and a water-soluble polymer, said at least one heat-insulation layer being provided between the support and the at least one receptor layer.

Other and further features and advantages of the invention will appear more fully from the following description.

#### DETAILED DESCRIPTION OF THE INVENTION

According to the present invention, there is provided the following means:

(1) A heat-sensitive transfer image-receiving sheet, comprising;

a support;

at least one receptor layer containing at least two kinds of latex polymers, said latex polymers having different elastic moduli from each other; and

at least one heat-insulation layer containing hollow latex polymer particles and a water-soluble polymer, said at least one heat-insulation layer being provided between the support and the at least one receptor layer;

(2) The heat-sensitive transfer image-receiving sheet according to the above item (1), wherein, among the latex polymers contained in the receptor layer, an elastic modulus of a latex polymer having the lowest elastic modulus is 1500 MPa or less, and an elastic modulus of a latex polymer having the highest elastic modulus is 1600 MPa or more, but 2200 MPa or less;

(3) The heat-sensitive transfer image-receiving sheet according to the above item (1) or (2), wherein the receptor layer includes an upper layer and a lower layer, and a latex-polymer composition of the upper layer is different from that of the lower layer;

(4) The heat-sensitive transfer image-receiving sheet according to the above item (3), wherein the upper layer comprises the latex polymer having the highest elastic modulus in a highest proportion; and the lower layer comprises the latex polymer having the lowest elastic modulus in a highest proportion;

(5) The heat-sensitive transfer image-receiving sheet according to any one of the above items (1) to (4), wherein at least one latex polymer contained in the receptor layer is a copolymer containing a repeating unit derived from vinyl chloride; and

(6) The heat-sensitive transfer image-receiving sheet according to any one of the above items (1) to (5), wherein the receptor layer and the heat insulation layer are simultaneously applied, in the production process of the heat-sensitive transfer image-receiving sheet.

The present invention is explained in detail below.

First, the heat-sensitive transfer image-receiving sheet (image-receiving sheet) of the present invention is explained.

The heat-sensitive transfer image-receiving sheet of the present invention is provided with at least one dye-receiving layer (receptor layer) and at least one heat insulation layer on a support. It is preferable to form an undercoat layer between the receptor layer and the support. As the undercoat layer, for example, a white background control layer, a charge control layer, an adhesive layer and a primer layer can be formed. Also, the heat insulation layer is preferably formed between the undercoat layer and the support. It is preferable that a curling control layer, a writing layer, or a charge-control layer be formed on the backside of the support. Each of these layers is applied using a usual method such as a roll coating, a bar coating, a gravure coating, a gravure reverse coating, a dye coating, a slide coating and a curtain coating. In practicing the present invention, a method capable of conducting a simultaneous multi-layer coating, such as the slide coating and the curtain coating, is preferable.

#### (Receptor Layer)

The receptor layer performs functions of receiving dyes transferred from an ink sheet and retaining images formed. The image-receiving sheet of the present invention has at least one receptor layer preferably containing at least one thermoplastic receiving polymer that can receive a dye.

The receiving polymer is preferably used, as it is dispersed in a water-soluble dispersion medium as a latex polymer. In addition, the receptor layer preferably contains a water-soluble polymer together with the latex polymer. Co-presence of the latex polymer and the water-soluble polymer allows presence of the water-soluble polymer, which is hardly dyable, among the latex polymers and prevents diffusion of the dye fixed on the latex polymer, and consequently, reduces changes in the color sharpness of the receptor layer with the lapse of time and forms a recorded image smaller in changes for its transferred image quality with the lapse of time.

The receptor layer may contain, in addition to the latex polymer of the receiving polymer, another latex polymer having a different function, for example, for the purpose of adjusting the elastic modulus of the film.

#### <Latex Polymer>

The latex polymer (polymer latex) used in the present invention is explained.

Latex polymers are described in "Gosei Jushi Emulsion (Synthetic Resin Emulsion)", compiled by Taira Okuda and Hiroshi Inagaki, issued by Kobunshi Kanko Kai (1978); "Gosei Latex no Oyo (Application of Synthetic Latex)", compiled by Takaaki Sugimura, Yasuo Kataoka, Souichi Suzuki, and Keishi Kasahara, issued by Kobunshi Kanko Kai (1993); Soichi Muroi, "Gosei Latex no Kagaku (Chemistry of Synthetic Latex)", issued by Kobunshi Kanko Kai (1970); Yoshiaki Miyosawa (supervisor) "Suisei Coating-Zairyō no Kaihatsu to Oyo (Development and Application of Aqueous Coating Material)", issued by CMC Publishing Co., Ltd. (2004) and JP-A-64-538, and so forth.

In the heat-sensitive transfer image-receiving sheet of the present invention, the latex polymer used in the receptor layer is a dispersion in which water-insoluble hydrophobic polymers are dispersed as fine particles in a water-soluble dispersion medium. The latex polymer is not particularly limited, but hydrophobic polymers such as vinyl chlorides, acrylic-series polymers, polyesters, rubbers (e.g., SBR resins), polyurethanes, polyvinyl chlorides, polyvinyl acetates, polyvinylidene chlorides, and polyolefins, are preferably used. Among these, vinyl chlorides, acrylic-series polymers, rubbers (e.g., SBR resins), and polyvinyl acetates are more preferable. In the present invention, the receptor layer contains at least two latex polymers having different elastic moduli from each other.

In the present invention, the elastic modulus is measured according to a testing method for tensile properties of plastics. A specific method is explained below. At first, latex polymers are freeze dried to make them a powder. The thus-obtained latex polymer powder is processed to a polymer sheet having a uniform thickness of 200  $\mu\text{m}$  using a temperature-controllable contact bonding press machine. Then, a 5 cm $\times$ 1 cm long fragment is cut off from the polymer sheet to use it as a sample. Subsequently, the sample is subjected to a tensile test under the conditions of 25°C., 3 mm/min tensile speed, and 30 mm distance between grips. The elastic modulus is calculated from the data obtained by measurement.

Described below is a preferable range of the elastic modulus of the latex polymers having different elastic moduli from each other that are used in the present invention. The elastic modulus of the latex polymer having the lowest elastic modulus is preferably 1500 MPa or less, and more preferably 1300

MPa or less. On the other hand, the elastic modulus of the latex polymer having the highest elastic modulus is preferably 1600 MPa or more but 2200 MPa or less, and more preferably 1600 MPa or more but 2000 MPa or less.

In the present invention, two or more latex polymers having different elastic moduli from each other are contained in the receptor layer. It is more preferable that there is a difference in the type and the used amount of the latex polymers forming a receptor layer between an upper layer and a lower layer of the receptor layer. Herein, the term "upper layer of the receptor layer" means, in the heat-sensitive transfer image-receiving sheet, the side of the receptor layer that contacts with an ink sheet at the time of image formation. On the other hand, the term "lower layer of the receptor layer" herein means the side of the receptor layer that does not contact with an ink sheet, namely the side of the receptor layer that is closest to a heat insulating layer (or a support).

The phrase "there is a difference in the type of the latex polymers" herein means that a monomer type of the repeating unit forming the latex polymer may be different between latex polymers, and/or a ratio of monomer composition may be different between latex polymers.

In the present invention, it is preferable to incorporate the latex polymer having a relatively high elastic modulus in the upper layer of the receptor layer. A preferable ratio of such the latex polymer is 50% or more, and more preferably 70% or more, based on the total amount of the latex polymers contained in the upper layer of the receptor layer. Of the latex polymers that can be used in the upper layer of the receptor layer, preferred are latex polymers having high affinity for dyes. Specifically, it is preferable to use hydrophobic polymers such as vinyl chloride-based polymers, acrylate-based polymers, polyesters, rubbers (e.g., SBR resins), polyurethanes, polyvinyl chlorides, polyvinyl acetates, polyvinylidene chlorides, and polyolefins, as mentioned above. Incorporation of the latex polymer having both relatively high elastic modulus and high affinity for a dye in the upper layer of the receptor layer makes it possible to provide a resistance to damage from scratches on the surface of the heat-sensitive transfer image-receiving sheet, and also to obtain a sufficient image-transfer density.

In the present invention, it is preferable to incorporate the latex polymer having a relatively low elastic modulus in the lower layer of the receptor layer. A preferable ratio of such the latex polymer is 50% or more, and more preferably 70% or more, based on the total amount of the latex polymers contained in the lower layer of the receptor layer. Of the latex polymers that can be used in the lower layer of the receptor layer, preferred are latex polymers having a low elastic modulus. Specifically, it is preferable to use hydrophobic polymers such as vinyl chloride-based polymers, acrylate-based polymers, polyesters, rubbers (e.g., SBR resins), polyurethanes, polyvinyl chlorides, polyvinyl acetates, polyvinylidene chlorides, and polyolefins, as mentioned above. The use of the lower layer of the receptor layer composed of latex polymer having a relatively low elastic modulus makes it possible to compensate lack of cushion characteristics (cushion properties) that occurs owing to the hardness of the interlayer (heat-insulating layer) containing hollow polymer particles.

In the heat-sensitive transfer image-receiving sheet of the present invention, as the latex polymer used in the receptor layer, a vinyl chloride-based polymer (a copolymer containing a repeating unit derived from vinyl chloride) is particularly preferred. In synthesis of the vinyl chloride-series latex polymers containing a vinyl chloride as a monomer unit that can be used in the present invention, there is no particular limitation to other monomers that can be used in combination

with the vinyl chloride monomer, and the following monomer groups (a) to (j) may be preferably used as those polymerizable in a usual radical polymerization or ion polymerization method. These monomers may be selected singly or combined freely to synthesize the latex polymer.

—Monomer Groups (a) to (j)—

- (a) Conjugated dienes: 1,3-pentadiene, isoprene, 1-phenyl-1,3-butadiene, 1- $\alpha$ -naphthyl-1,3-butadiene, 1- $\beta$ -naphthyl-1,3-butadiene, cyclopentadiene, etc.
- (b) Olefins: ethylene, propylene, vinyl chloride, vinylidene chloride, 6-hydroxy-1-hexene, 4-pentenoic acid, methyl 8-nonenate, vinylsulfonic acid, trimethylvinylsilane, trimethoxyvinylsilane, 1,4-divinylcyclohexane, 1,2,5-trivinylcyclohexane, etc.
- (c)  $\alpha,\beta$ -unsaturated carboxylates: alkyl acrylates, such as methyl acrylate, ethyl acrylate, butyl acrylate, cyclohexyl acrylate, 2-ethylhexyl acrylate, and dodecyl acrylate; substituted alkyl acrylates, such as 2-chloroethyl acrylate, benzyl acrylate, and 2-cyanoethyl acrylate; alkyl methacrylates, such as methyl methacrylate, butyl methacrylate, 2-ethylhexyl methacrylate, and dodecyl methacrylate; substituted alkyl methacrylates, such as 2-hydroxyethyl methacrylate, glycidyl methacrylate, glycerin monomethacrylate, 2-acetoxyethyl methacrylate, tetrahydrofurfuryl methacrylate, 2-methoxyethyl methacrylate, polypropylene glycol monomethacrylates (mole number of added polyoxypropylene=2 to 100), 3-N,N-dimethylaminopropyl methacrylate, chloro-3-N,N,N-trimethylammoniopropyl methacrylate, 2-carboxyethyl methacrylate, 3-sulfopropyl methacrylate, 4-oxysulfonylpropyl methacrylate, 3-trimethoxysilylpropyl methacrylate, allyl methacrylate, and 2-isocyanatoethyl methacrylate; derivatives of unsaturated dicarboxylic acids, such as monobutyl maleate, dimethyl maleate, monomethyl itaconate, and dibutyl itaconate; multifunctional esters, such as ethylene glycol diacrylate, ethylene glycol dimethacrylate, 1,4-cyclohexane diacrylate, pentaerythritol tetramethacrylate, pentaerythritol triacrylate, trimethylolethane triacrylate, trimethylolethane triacrylate, dipentaerythritol pentamethacrylate, pentaerythritol hexaacrylate, and 1,2,4-cyclohexane tetramethacrylate; etc.
- (d)  $\alpha,\beta$ -unsaturated carboxylic amides: acrylamide, methacrylamide, N-methylacrylamide, N,N-dimethylacrylamide, N-methyl-N-hydroxyethylmethacrylamide, N-tert-butylacrylamide, N-tert-octylmethacrylamide, N-cyclohexylacrylamide, N-phenylacrylamide, N-(2-acetoxyethyl)acrylamide, N-acryloylmorpholine, diacetone acrylamide, itaconic diamide, N-methylmaleimide, 2-acrylamide-methylpropane sulfonic acid, methylenebisacrylamide, dimethacryloylpiperazine, etc.
- (e) Unsaturated nitriles: acrylonitrile, methacrylonitrile, etc.
- (f) Styrene and derivatives thereof: styrene, vinyltoluene, p-tert-butylstyrene, vinylbenzoic acid, methyl vinylbenzoate, ac-methylstyrene, p-chloromethylstyrene, vinylnaphthalene, p-hydroxymethylstyrene, sodium p-styrenesulfonate, potassium p-styrenesulfinate, p-aminomethylstyrene, 1,4-divinylbenzene, etc.
- (g) Vinyl ethers: methyl vinyl ether, butyl vinyl ether, methoxyethyl vinyl ether, etc.
- (h) Vinyl esters: vinyl acetate, vinyl propionate, vinyl benzoate, vinyl salicylate, vinyl chloroacetate, etc.
- (i)  $\alpha,\beta$ -unsaturated carboxylic acids and salts thereof: acrylic acid, methacrylic acid, itaconic acid, maleic acid, sodium acrylate, ammonium methacrylate, potassium itaconate, etc.
- (j) Other polymerizable monomers: N-vinylimidazole, 4-vinylpyridine, N-vinylpyrrolidone, 2-vinylloxazoline, 2-isopropenylloxazoline, divinylsulfone, etc.

These polymers may be straight-chain, branched, or cross-linked polymers, the so-called homopolymers obtained by polymerizing single type of monomers, or copolymers obtained by polymerizing two or more types of monomers. In the case of the copolymers, these copolymers may be either random copolymers or block copolymers. The molecular weight of each of these polymers is preferably 5,000 to 1,000,000, and further preferably 10,000 to 500,000 in terms of number average molecular weight. Polymers having excessively small molecular weight impart insufficient dynamic strength to the layer containing the latex, and polymers having excessively large molecular weight bring about poor filming ability, and therefore both cases are not preferable. Crosslinkable latex polymers are also preferably used.

The latex polymer in the other structure that can be used in combination with the latex polymer comprising vinyl chloride as a monomer unit is not particularly limited, but hydrophobic polymers such as acrylic-series polymers, polyesters, rubbers (e.g., SBR resins), polyurethanes, polyvinyl chlorides, polyvinyl acetates, polyvinylidene chlorides, and polyolefins, are preferably used. These polymers may be straight-chain, branched, or cross-linked polymers, the so-called homopolymers obtained by polymerizing single type of monomers, or copolymers obtained by polymerizing two or more types of monomers. In the case of the copolymers, these copolymers may be either random copolymers or block copolymers. The molecular weight of each of these polymers is preferably 5,000 to 1,000,000, and further preferably 10,000 to 500,000 in terms of number average molecular weight. A polymer having an excessively small molecular weight imparts insufficient dynamic strength to a layer containing a latex of the polymer, and a polymer having an excessively large molecular weight brings about poor filming ability, and therefore both cases are not preferable. Crosslinkable polymer latexes are also preferably used.

The latex polymer for use in the present invention may be latex of the so-called core/shell type, other than ordinary latex polymer of a uniform structure. When using a core/shell type latex polymer, it is preferred in some cases that the core and the shell have different glass transition temperatures. The glass transition temperature (Tg) of the latex polymer for use in the present invention is preferably -30°C. to 100°C., more preferably 0°C. to 80°C., further more preferably 10°C. to 70°C., and especially to 60°C.

The glass transition temperature (Tg) is calculated according to the following equation:

$$1/Tg = \sum (Xi/Tgi)$$

wherein, assuming that the polymer is a copolymer composed of n monomers from i=1 to i=n, Xi is a weight fraction of the i-th monomer ( $\sum Xi = 1$ ) and Tgi is glass transition temperature (measured in absolute temperature) of a homopolymer formed from the i-th monomer. The symbol  $\Sigma$  means the sum of i=1 to i=n. The value of the glass transition temperature of a homopolymer formed from each monomer (Tgi) is adopted from J. Brandrup and E. H. Immergut, "Polymer Handbook, 3rd. Edition", Wiley-Interscience (1989).

The glass transition temperature (Tg) of the latex polymer having the other structure that can be used in combination with the latex polymer comprising vinyl chloride as a monomer unit is preferably in the range of -30°C. to 100°C., more preferably 0°C. to 80°C., still more preferably 20°C. to 70°C., in view of film-forming properties (brittleness for working) and image preservability. A blend of two or more types of polymers can be used as the binder. When a blend of two or more polymers is used, the average Tg obtained by summing up the Tg of each polymer weighted by its proportion, is

preferably within the foregoing range. Also, when phase separation occurs or when a core-shell structure is adopted, the weighted average Tg is preferably within the foregoing range.

- 5 The latex polymer for use in the present invention preferably has a minimum film-forming temperature (MFT) of from -30 to 90°C., more preferably from 0 to 70°C. In order to control the minimum film-forming temperature, a film-forming aid may be added. The film-forming aid is also called 10 a temporary plasticizer, and it is an organic compound (usually an organic solvent) that reduces the minimum film-forming temperature of a latex polymer. It is described in, for example, Souichi Muroi, "Gosei Latex no Kagaku (Chemistry of Synthetic Latex)", issued by Kobunshi Kanko Kai 15 (1970). Preferable examples of the film-forming aid are listed below, but the compounds that can be used in the present invention are not limited to the following specific examples.

- Z-1: Benzyl alcohol  
Z-2: 2,2,4-Trimethylpentanediol-1,3-monoisobutyrate  
20 Z-3: 2-Dimethylaminoethanol  
Z-4: Diethylene glycol

The latex polymer comprising a copolymer having repeating units derived from vinyl chloride that can be used in the present invention is commercially available, and polymers described below may be utilized. Examples thereof include 25 G351 and G576 (trade names, manufactured by Nippon Zeon Co., Ltd.); VINYBLAN 240, 270, 277, 375, 386, 609, 550, 601, 602, 630, 660, 671, 683, 680, 680S, 681N, 685R, 277, 380, 381, 410, 430, 432, 860, 863, 865, 867, 900, 900GT, 30 938 and 950 (trade names, manufactured by Nissin Chemical Industry Co., Ltd.).

The latex polymer in the other structure that can be used in combination with the latex polymer having repeating units derived from vinyl chloride is also commercially available, 35 and polymers described below may be utilized in combination. Examples of the acrylic-series polymers include Cevian A-4635, 4718, and 4601 (trade names, manufactured by Daicel Chemical Industries); Nipol Lx811, 814, 821, 820, 855 (P-17: Tg 36°C.), and 857x2 (P-18: Tg 43°C.) (trade 40 names, manufactured by Nippon Zeon Co. Voncoat R3370 (P-19: Tg 25°C.), and 4280 (P-20: Tg 15°C.) (trade names, manufactured by Dai-Nippon Ink & Chemicals, Inc.); Julimer ET-410 (P-21: Tg 44°C.) (trade name, manufactured by Nihon Junyaku K.K.); AE116 (P-22: Tg 50°C.), AE119 (P-23: Tg 55°C.), AE121 (P-24: Tg 58°C.), AE125 (P-25: Tg 60°C.), AE134 (P-26: Tg 48°C.), AE137 (P-27: Tg 48°C.), 45 AE140 (P-28: Tg 53°C.), and AE173 (P-29: Tg 60°C.) (trade names, manufactured by JSR Corporation); Aron A-104 (P-30: Tg 45°C.) (trade name, manufactured by Toagosei Co., Ltd.); NS-600X, and NS-620X (trade names, manufactured by Takamatsu Yushi K.K.); VINYBLAN 2580, 2583, 2641, 2770, 2770H, 2635, 2886, 5202C, and 2706 (trade 50 names, manufactured by Nissin Chemical Industry Co., Ltd.).

Examples of the polyesters include FINETEX ES650, 611, 55 675, and 850 (trade names, manufactured by Dainippon Ink and Chemicals, Incorporated); WD-size, and WMS (trade names, manufactured by Eastman Chemical Ltd.); A-110, A-115GE, A-120, A-121, A-124GP, A-124S, A-160P, A-210, A-215GE, A-510, A-513E, A-515GE, A-520, A-610, A-613, 60 A-615GE, A-620, WAC-10, WAC-15, WAC-17XC, WAC-20, S-110, S-110EA, S-111SL, S-120, S-140, S-140A, S-250, S-252G, S-250S, S-320, S-680, DNS-63P, NS-122L, NS-122LX, NS-244LX, NS-140L, NS-141LX, and NS-282LX (trade names, manufactured by Takamatsu Yushi K.K.); Aronmelt PES-1000 series, and PES-2000 series (trade names, manufactured by Toagosei Co., Ltd.); Bironal 65 MD-1100, MD-1200, MD-1220, MD-1245, MD-1250,

MD-1335, MD-1400, MD-1480, MD-1500, MD-1930, and MD-1985 (trade names, manufactured by Toyobo Co., Ltd.); and Ceporjon ES (trade name, manufactured by Sumitomo Seika Chemicals Co., Ltd.).

Examples of the polyurethanes include HYDRAN AP10, AP20, AP30, AP40, and 101H, Vondic 1320NS and 1610NS (trade names, manufactured by Dainippon Ink and Chemicals, Incorporated); D-1000, D-2000, D-6000, D-4000, and D-9000 (trade names, manufactured by Dainichi Seika Color & Chemicals Mfg. Co., Ltd.); NS-155X, NS-310A, NS-310X, and NS-311X (trade names, manufactured by Takamatsu Yushi K.K.); Elastron (trade name, manufactured by Dai-ichi Kogyo Seiyaku Co., Ltd.).

Examples of the rubbers include LACSTAR 7310K, 3307B, 4700H, and 7132C (trade names, manufactured by Dainippon Ink & Chemicals Incorporated); Nipol Lx416, LX410, LX430, LX435, LX110, LX415A, LX438C, 2507H, LX303A, LX407BP series, V1004, and MH5055 (trade names, manufactured by Nippon Zeon Co., Ltd.).

Examples of the polyolefins include Chemipearl S120, SA100, and V300 (P-40: Tg 80° C.) (trade names, manufactured by Mitsui Petrochemical); Voncoat 2830, 2210, and 2960 (trade names, manufactured by Dainippon Ink and Chemicals, Incorporated); Zaikusen and Ceporjon G (trade names, manufactured by Sumitomo Seika Chemicals Co., Ltd.).

Examples of the copolymer nylons include Ceporjon PA (trade name, manufactured by Sumitomo Seika Chemicals Co., Ltd.).

Examples of the polyvinyl acetates include VINYBLAN 1080, 1082, 1085W, 1108W, 1108S, 1563M, 1566, 1570, 1588C, A22J7-F2, 1128C, 1137, 1138, A20J2, A23J1, A23J1, A23K1, A23P2E, A68J1N, 1086A, 1086, 1086D, 1108S, 1187, 1241LT, 1580N, 1083, 1571, 1572, 1581, 4465, 4466, 4468W, 4468S, 4470, 4485LL, 4495LL, 1023, 1042, 1060, 1060S, 1080M, 1084W, 1084S, 1096, 1570K, 1050, 1050S, 3290, 1017AD, 1002, 1006, 1008, 1107L, 1225, 1245L, GV-6170, GV-6181, 4468W, and 4468S (trade names, manufactured by Nissin Chemical Industry Co., Ltd.).

These latex polymers may be used singly, or two or more of these polymers may be blended, if necessary.

In the receptor layer for use in the present invention, a ratio of the latex polymer comprising a component of vinyl chloride is preferably 50 mass % or more of the whole solid content in the layer.

The dispersed state may be one in which polymer is emulsified in a dispersion medium, one in which polymer underwent emulsion polymerization, one in which polymer underwent micelle dispersion, one in which polymer molecules partially have a hydrophilic structure and thus the molecular chains themselves are dispersed in a molecular state, or the like.

The latex polymer for use in the present invention can be easily obtained by a solution polymerization method, a suspension polymerization method, an emulsion polymerization method, a dispersion polymerization method, an anionic polymerization method, a cationic polymerization method, or the like. Above all, an emulsion polymerization method in which the polymer is obtained as a latex is the most preferable. Also, a method is preferable in which the polymer is prepared in a solution, and the solution is neutralized, or an emulsifier is added to the solution, to which water is then added, to prepare an aqueous dispersion by forced stirring. For example, an emulsion polymerization method comprises conducting polymerization under stirring at about 30° C. to about 100° C. (preferably 60° C. to 90° C.) for 3 to 24 hours by using water or a mixed solvent of water and a water-

miscible organic solvent (such as methanol, ethanol, or acetone) as a dispersion medium, a monomer mixture in an amount of 5 mass % to 150 mass % based on the amount of the dispersion medium, an emulsifier and a polymerization initiator. Various conditions such as the dispersion medium, the monomer concentration, the amount of initiator, the amount of emulsifier, the amount of dispersant, the reaction temperature, and the method for adding monomers are suitably determined considering the type of the monomers to be used. Furthermore, it is preferable to use a dispersant when necessary.

Generally, the emulsion polymerization method can be conducted according to the disclosures of the following documents: "Gosei Jushi Emarujon (Synthetic Resin Emulsions)" (edited by Taira Okuda and Hiroshi Inagaki and published by Kobunshi Kankokai (1978)); "Gosei Ratekkusu no Oyo (Applications of Synthetic Latexes)" (edited by Takaaki Sugimura, Yasuo Kataoka, Soichi Suzuki, and Keiji Kasahara and published by Kobunshi Kankokai (1993)); and "Gosei Ratekkusu no Kagaku (Chemistry of Synthetic Latexes)" (edited by Soichi Muroi and published by Kobunshi Kankokai (1970)). The emulsion polymerization method for synthesizing the latex polymer for use in the present invention may be a batch polymerization method, a monomer (continuous or divided) addition method, an emulsion addition method, or a seed polymerization method. The emulsion polymerization method is preferably a batch polymerization method, a monomer (continuous or divided) addition method, or an emulsion addition method in view of the productivity of latex.

The polymerization initiator may be any polymerization initiator having radical generating ability. The polymerization initiator to be used may be selected from inorganic peroxides such as persulfates and hydrogen peroxide, peroxides described in the organic peroxide catalogue of NOF Corporation, and azo compounds as described in the azo polymerization initiator catalogue of Wako Pure Chemical Industries, Ltd. Among them, water-soluble peroxides such as persulfates and water-soluble azo compounds as described in the azo polymerization initiator catalogue of Wako Pure Chemical Industries, Ltd. are preferable; ammonium persulfate, sodium persulfate, potassium persulfate, azobis(2-methylpropionamidine) hydrochloride, azobis(2-methyl-N-(2-hydroxyethyl)propionamide), and azobiscyanovaleric acid are more preferable; and peroxides such as ammonium persulfate, sodium persulfate, and potassium persulfate are especially preferable from the viewpoints of image preservability, solubility, and cost.

The amount of the polymerization initiator to be added is, based on the total amount of monomers, preferably 0.3 mass % to 2.0 mass %, more preferably 0.4 mass % to 1.75 mass %, and especially preferably 0.5 mass % to 1.5 mass %.

The polymerization emulsifier to be used may be selected from anionic surfactants, nonionic surfactants, cationic surfactants, and ampholytic surfactants. Among them, anionic surfactants are preferable from the viewpoints of dispersibility and image preservability. Sulfonic acid type anionic surfactants are more preferable because polymerization stability can be ensured even with a small addition amount and they have resistance to hydrolysis. Long chain alkylphenyl ether disulfonic acid salts (whose typical example is PELEX SS-H (trade name) manufactured by Kao Corporation) are still more preferable, and low electrolyte types such as PIONIN A-43-S (trade name, manufactured by Takemoto Oil & Fat Co., Ltd.) are especially preferable.

The amount of sulfonic acid type anionic surfactant as the polymerization emulsifier is preferably 0.1 mass % to 10.0

## 11

mass %, more preferably 0.2 mass % to 7.5 mass %, and especially preferably 0.3 mass % to 5.0 mass %, based on the total amount of monomers.

It is preferable to use a chelating agent in synthesizing the latex polymer to be used in the present invention. The chelating agent is a compound capable of coordinating (chelating) a polyvalent ion such as metal ion (e.g., iron ion) or alkaline earth metal ion (e.g., calcium ion), and examples of the chelate compound which can be used include the compounds described in JP-B-6-8956 ("JP-B" means examined Japanese patent publication), U.S. Pat. No. 5,053,322, JP-A-4-73645, JP-A-4-127145, JP-A-4-247073, JP-A-4-305572, JP-A-6-11805, JP-A-5-173312, JP-A-5-66527, JP-A-5-158195, JP-A-6-118580, JP-A-6-110168, JP-A-6-161054, JP-A-6-175299, JP-A-6-214352, JP-A-7-114161, JP-A-7-114154, JP-A-7-120894, JP-A-7-199433, JP-A-7-306504, JP-A-9-43792, JP-A-8-314090, JP-A-10-182571, JP-A-10-182570, and JP-A-11-190892.

Preferred examples of the chelating agent include inorganic chelate compounds (e.g., sodium tripolyphosphate, sodium hexametaphosphate, sodium tetrapolyphosphate), aminopolycarboxylic acid-based chelate compounds (e.g., nitrilotriacetic acid, ethylenediaminetetraacetic acid), organic phosphonic acid-based chelate compounds (e.g., compounds described in Research Disclosure, No. 18170, JP-A-52-102726, JP-A-53-42730, JP-A-56-97347, JP-A-54-121127, JP-A-55-4024, JP-A-55-4025, JP-A-55-29883, JP-A-55-126241, JP-A-55-65955, JP-A-55-65956, JP-A-57-179843, JP-A-54-61125, and West German Patent No. 1045373), polyphenol-based chelating agents, and polyamine-based chelate compounds, with aminopolycarboxylic acid derivatives being particularly preferred.

Preferred examples of the aminopolycarboxylic acid derivative include the compounds shown in the Table attached to "EDTA (—Complexane no Kagaku—) (EDTA—Chemistry of Complexane)", Nankodo (1977). In these compounds, a part of the carboxyl groups may be substituted by an alkali metal salt such as sodium or potassium or by an ammonium salt. More preferred examples of the aminopolycarboxylic acid derivative include iminodiacetic acid, N-methyliminodiacetic acid, N-(2-aminoethyl)iminodiacetic acid, N-(carbamoylmethyl)iminodiacetic acid, nitrilotriacetic acid, ethylenediamine-N,N'-diacetic acid, ethylenediamine-N,N'-di- $\alpha$ -propionic acid, ethylenediamine-N,N'-di- $\beta$ -propionic acid, N,N'-ethylene-bis( $\alpha$ -o-hydroxyphenyl)glycine, N,N'-di(2-hydroxybenzyl)ethylenediamine-N,N'-diacetic acid, ethylenediamine-N,N'-diacetic acid-N,N'-diacetohydroxamic acid, N-hydroxyethylethylenediamine-N,N',N'-triacetic acid, ethylenediamine-N,N,N',N'-tetraacetic acid, 1,2-propylenediamine-N,N,N',N'-tetraacetic acid, d,1-2,3-diaminobutane-N,N,N',N'-tetraacetic acid, meso-2,3-diaminobutane-N,N,N',N'-tetraacetic acid, 1-phenylethylenediamine-N,N,N',N'-tetraacetic acid, d,1-1,2-diphenylethylenediamine-N,N,N',N'-tetraacetic acid, 1,4-diaminobutane-N,N,N',N'-tetraacetic acid, trans-cyclobutane-1,2-diamine-N,N,N',N'-tetraacetic acid, trans-cyclopentane-1,2-diamine-N,N,N',N'-tetraacetic acid, trans-cyclohexane-1,2-diamine-N,N,N',N'-tetraacetic acid, cis-cyclohexane-1,2-diamine-N,N,N',N'-tetraacetic acid, cyclohexane-1,3-diamine-N,N,N',N'-tetraacetic acid, cyclohexane-1,4-diamine-N,N,N',N'-tetraacetic acid, o-phenylenediamine-N,N,N',N'-tetraacetic acid, cis-1,4-diaminobutene-N,N,N',N'-tetraacetic acid, trans-1,4-diaminobutene-N,N,N',N'-tetraacetic acid,  $\alpha$ , $\alpha$ '-diamino-oxylen-N,N,N',N'-tetraacetic acid, 2-hydroxy-1,3-propanediamine-N,N,N',N'-tetraacetic acid, 2,2'-oxy-bis(ethyliminodiacetic acid), 2,2'-ethylenedioxy-bis

## 12

(ethyliminodiacetic acid), ethylenediamine-N,N'-diacetic acid-N,N'-di- $\alpha$ -propionic acid, ethylenediamine-N,N'-diacetic acid-N,N'-di- $\beta$ -propionic acid, ethylenediamine-N,N,N',N'-pentaacetic acid, diethylenetriamine-N,N,N',N'',N'''-pentaacetic acid, triethylenetetramine-N,N,N',N'',N'''-hexaacetic acid, and 1,2,3-triaminopropane-N,N,N',N'',N'''-hexaacetic acid. In these compounds, a part of the carboxyl groups may be substituted by an alkali metal salt such as sodium or potassium or by an ammonium salt.

10 The amount of the chelating agent to be added is preferably 0.01 mass % to 0.4 mass %, more preferably 0.02 mass % to 0.3 mass %, and especially preferably 0.03 mass % to 0.15 mass %, based on the total amount of monomers. When the addition amount of the chelating agent is too small, metal ions entering during the preparation of the latex polymer are not sufficiently trapped, and the stability of the latex against aggregation is lowered, whereby the coating properties become worse. When the amount is too large, the viscosity of the latex increases, whereby the coating properties are lowered.

15 In the preparation of the latex polymer to be used in the present invention, it is preferable to use a chain transfer agent. As the chain transfer agent, ones described in Polymer Handbook (3rd Edition) (Wiley-Interscience, 1989) are preferable. Sulfur compounds are more preferable because they have high chain-transfer ability and because the required amount is small. Especially, hydrophobic mercaptane-based chain transfer agents such as tert-dodecylmercaptane and n-dodecylmercaptane are preferable.

20 The amount of the chain transfer agent to be added is preferably 0.2 mass % to 2.0 mass %, more preferably 0.3 mass % to 1.8 mass %, and especially preferably 0.4 mass % to 1.6 mass %, based on the total amount of monomers.

25 Besides the foregoing compounds, in the emulsion polymerization, use can be made of additives, such as electrolytes, stabilizers, thickeners, defoaming agents, antioxidants, vulcanizers, antifreezing agents, gelling agents, and vulcanization accelerators, as described, for example, in Synthetic Rubber Handbook.

30 In the present invention, it is preferable to prepare the latex polymer by applying an aqueous type coating solution and then drying it. The "aqueous type" so-called here means that 60% by mass or more of the solvent (dispersion medium) of the coating solution is water. As a component other than water 35 in the coating solution, a water miscible organic solvent may be used, such as methyl alcohol, ethyl alcohol, isopropyl alcohol, methyl cellosolve, ethyl cellosolve, dimethylformamide, ethyl acetate, diacetone alcohol, furfuryl alcohol, benzyl alcohol, diethylene glycol monoethyl ether, and oxyethyl phenyl ether.

40 The latex polymer in the image-receiving sheet used in the present invention includes a state of a gel or dried film formed by removing a part of solvents by drying after coating.  
<Water-Soluble Polymer>

45 The receptor layer preferably contains a water-soluble polymer. Herein, "water-soluble polymer" means a polymer which dissolves, in 100 g water at 20° C., in an amount of preferably 0.05 g or more, more preferably 0.1 g or more, further preferably 0.5 g or more, and particularly preferably 1 g or more. The water-soluble polymer which can be used in the present invention is natural polymers (polysaccharide type, microorganism type, and animal type), semi-synthetic polymers (cellulose-based, starch-based, and alginic acid-based), and synthetic polymer type (vinyl type and others); and synthetic polymers including polyvinyl alcohols, and natural or semi-synthetic polymers using celluloses derived from plant as starting materials, which will be explained later,

correspond to the water-soluble polymer usable in the present invention. The latex polymers recited above are not included in the water-soluble polymers which can be used in the present invention. In the present invention, the water-soluble polymer is also referred to as a binder, for differentiation from the latex polymer described above.

Among the water-soluble polymers which can be used in the present invention, the natural polymers and the semi-synthetic polymers will be explained in detail. Specific examples include the following polymers: plant type polysaccharides such as gum arabics,  $\kappa$ -carrageenans, t-carrageenans,  $\lambda$ -carrageenans, guar gums (e.g. Supercol, manufactured by Squalon), locust bean gums, pectins, tragacanths, corn starches (e.g. Purity-21, manufactured by National Starch & Chemical Co.), and phosphorylated starches (e.g. National 78-1898, manufactured by National Starch & Chemical Co.); microbial type polysaccharides such as xanthan gums (e.g. Keltrol T, manufactured by Kelco) and dextrans (e.g. Nadex 360, manufactured by National Starch & Chemical Co.); animal type natural polymers such as gelatins (e.g. Crodyne B419, manufactured by Croda), caseins, sodium chondroitin sulfates (e.g. Cromoist CS, manufactured by Croda); cellulose-based polymers such as ethylcelluloses (e.g. Cellofas WLD, manufactured by I.C.I.), carboxymethylcelluloses (e.g. CMC, manufactured by Daicel), hydroxyethylcelluloses (e.g. HEC, manufactured by Daicel), hydroxypropylcelluloses (e.g. Klucel, manufactured by Aqualon), methylcelluloses (e.g. Viscontran, manufactured by Henkel), nitrocelluloses (e.g. Isopropyl Wet, manufactured by Hercules), and cationated celluloses (e.g. Crodacel QM, manufactured by Croda); starches such as phosphorylated starches (e.g. National 78-1898, manufactured by National Starch & Chemical Co.); alginic acid-based compounds such as sodium alginates (e.g. Keltone, manufactured by Kelco) and propylene glycol alginates; and other polymers such as cationated guar gums (e.g. Hi-care 1000, manufactured by Alcolac) and sodium hyaluronates (e.g. Hyalure, manufactured by Lifecare Biomedical) (all of the names are trade names).

Gelatin is one of preferable embodiments in the present invention. Gelatin having a molecular weight of from 10,000 to 1,000,000 may be used in the present invention. Gelatin that can be used in the present invention may contain an anion such as  $\text{Cl}^-$  and  $\text{SO}_4^{2-}$ , or alternatively a cation such as  $\text{Fe}^{2+}$ ,  $\text{Ca}^{2+}$ ,  $\text{Mg}^{2+}$ ,  $\text{Sn}^{2+}$ , and  $\text{Zn}^{2+}$ . Gelatin is preferably added as an aqueous solution.

Among the water-soluble polymers which can be used in the present invention, the synthetic polymers will be explained in detail. Examples of the acryl type include sodium polyacrylates, polyacrylic acid copolymers, polyacrylamides, polyacrylamide copolymers, and polydiethylaminoethyl(meth)acrylate quaternary salts or their copolymers. Examples of the vinyl type include polyvinylpyrrolidones, polyvinylpyrrolidone copolymers, and polyvinyl alcohols. Examples of the others include polyethylene glycols, polypropylene glycols, polyisopropylacrylamides, polymethyl vinyl ethers, polyethyleneimines, polystyrenesulfonic acids or their copolymers, naphthalenesulfonic acid condensate salts, polyvinylsulfonic acids or their copolymers, polyacrylic acids or their copolymers, acrylic acid or its copolymers, maleic acid copolymers, maleic acid monoester copolymers, acryloylmethylpropane-sulfonic acid or its copolymers, polydimethylallylaminium chlorides or their copolymers, polyamidines or their copolymers, polyimidazolines, dicyanamide type condensates, epichlorohydrin/dimethylamine condensates, Hofmann decomposed products of polyacrylamides, and water-soluble polyesters (Plascoat Z-221, Z-446, Z-561, Z-450,

Z-565, Z-850, Z-3308, RZ-105, RZ-570, Z-730 and RZ-142 (all of these names are trade names), manufactured by Goo Chemical Co., Ltd.).

In addition, highly-water-absorptive polymers, namely, homopolymers of vinyl monomers having  $-\text{COOM}$  or  $-\text{SO}_3\text{M}$  (M represents a hydrogen atom or an alkali metal atom) or copolymers of these vinyl monomers among them or with other vinyl monomers (for example, sodium methacrylate, ammonium methacrylate, Sumikagel L-5H (trade name) manufactured by Sumitomo Chemical Co., Ltd.) as described in, for example, U.S. Pat. No. 4,960,681 and JP-A-62-245260, may also be used.

Among the water-soluble synthetic polymers that can be used in the present invention, polyvinyl alcohols are preferable. The polyvinyl alcohols are explained in detail below.

Examples of completely saponified polyvinyl alcohol include PVA-105 [polyvinyl alcohol (PVA) content: 94.0 mass % or more; degree of saponification:  $98.5\pm0.5$  mol %; content of sodium acetate: 1.5 mass % or less; volatile constituent: 5.0 mass % or less; viscosity (4 mass %; 20° C.): 5.6 $\pm$ 0.4 CPS]; PVA-110 [PVA content: 94.0 mass %; degree of saponification:  $98.5\pm0.5$  mol %; content of sodium acetate: 1.5 mass %; volatile constituent: 5.0 mass %; viscosity (4 mass %; 20° C.): 11.0 $\pm$ 0.8 CPS]; PVA-117 [PVA content: 94.0 mass %; degree of saponification:  $98.5\pm0.5$  mol %; content of sodium acetate: 1.0 mass %; volatile constituent: 5.0 mass %; viscosity (4 mass %; 20° C.): 28.0 $\pm$ 3.0 CPS]; PVA-117H [PVA content: 93.5 mass %; degree of saponification: 99.6 $\pm$ 0.3 mol %; content of sodium acetate: 1.85 mass %; volatile constituent: 5.0 mass %; viscosity (4 mass %; 20° C.): 29.0 $\pm$ 3.0 CPS]; PVA-120 [PVA content: 94.0 mass %; degree of saponification:  $98.5\pm0.5$  mol %; content of sodium acetate: 1.0 mass %; volatile constituent: 5.0 mass %; viscosity (4 mass %; 20° C.): 39.5 $\pm$ 4.5 CPS]; PVA-124 [PVA content: 94.0 mass %; degree of saponification:  $98.5\pm0.5$  mol %; content of sodium acetate: 1.0 mass %; volatile constituent: 5.0 mass %; viscosity (4 mass %; 20° C.): 60.0 $\pm$ 6.0 CPS]; PVA-124H [PVA content: 93.5 mass %; degree of saponification: 99.6 $\pm$ 0.3 mol %; content of sodium acetate: 1.85 mass %; volatile constituent: 5.0 mass %; viscosity (4 mass %; 20° C.): 61.0 $\pm$ 6.0 CPS]; PVA-CS [PVA content: 94.0 mass %; degree of saponification:  $97.5\pm0.5$  mol %; content of sodium acetate: 1.0 mass %; volatile constituent: 5.0 mass %; viscosity (4 mass %; 20° C.): 27.5 $\pm$ 3.0 CPS]; PVA-CST [PVA content: 94.0 mass %; degree of saponification: 96.0 $\pm$ 0.5 mol %; content of sodium acetate: 1.0 mass %; volatile constituent: 5.0 mass %; viscosity (4 mass %; 20° C.): 27.0 $\pm$ 3.0 CPS]; and PVA-HC [PVA content: 90.0 mass %; degree of saponification: 99.85 mol % or more; content of sodium acetate: 2.5 mass %; volatile constituent: 8.5 mass %; viscosity (4 mass %; 20° C.): 25.0 $\pm$ 3.5 CPS] (all trade names, manufactured by Kuraray Co., Ltd.), and the like.

Examples of partially saponified polyvinyl alcohol include PVA-203 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.): 3.4 $\pm$ 0.2 CPS]; PVA-204 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.): 3.9 $\pm$ 0.3 CPS]; PVA-205 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.): 5.0 $\pm$ 0.4 CPS]; PVA-210 [PVA content: 94.0 mass %; degree of saponification:  $88.0\pm1.0$  mol %; content of sodium acetate: 1.0 mass %; volatile constituent: 5.0 mass %; viscosity (4 mass %; 20° C.): 9.0 $\pm$ 1.0 CPS]; PVA-217 [PVA content: 94.0 mass %; degree

of saponification:  $88.0\pm1.0$  mol %; content of sodium acetate: 1.0 mass %; volatile constituent: 5.0 mass %; viscosity (4 mass %; 20° C.):  $22.5\pm2.0$  CPS]; PVA-220 [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $30.0\pm3.0$  CPS]; PVA-224 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.):  $44.0\pm4.0$  CPS]; PVA-228 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.):  $65.0\pm5.0$  CPS]; PVA-235 [PVA content: 94.0 mass %; degree of saponification:  $88.0\pm1.5$  mol %; content of sodium acetate: 1.0 mass %; volatile constituent: 5.0 mass %; viscosity (4 mass %; 20° C.):  $95.0\pm15.0$  CPS]; PVA-217EE [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $23.0\pm3.0$  CPS]; PVA-217E [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $23.0\pm3.0$  CPS]; PVA-220E [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $31.0\pm4.0$  CPS]; PVA-224E [PVA content: 94.0 mass %; degree of saponification:  $88.0\pm1.0$  mol %; content of sodium acetate: 1.0 mass %; volatile constituent: 5.0 mass %; viscosity (4 mass %; 20° C.):  $45.0\pm5.0$  CPS]; PVA-403 [PVA content: 94.0 mass %; degree of saponification:  $80.0\pm1.5$  mol %; content of sodium acetate: 1.0 mass %; volatile constituent: 5.0 mass %; viscosity (4 mass %; 20° C.):  $3.1\pm0.3$  CPS]; PVA-405 [PVA content: 94.0 mass %; degree of saponification:  $81.5\pm1.5$  mol %; content of sodium acetate: 1.0 mass %; volatile constituent: 5.0 mass %; viscosity (4 mass %; 20° C.):  $4.8\pm0.4$  CPS]; PVA-420 [PVA content: 94.0 mass %; degree of saponification:  $79.5\pm1.5$  mol %; content of sodium acetate: 1.0 mass %; volatile constituent: 5.0 mass %]; PVA-613 [PVA content: 94.0 mass %; degree of saponification:  $93.5\pm1.0$  mol %; content of sodium acetate: 1.0 mass %; volatile constituent: 5.0 mass %; viscosity (4 mass %; 20° C.):  $16.5\pm2.0$  CPS]; L-8 [PVA content: 96.0 mass %; degree of saponification:  $71.0\pm1.5$  mol %; content of sodium acetate: 1.0 mass % (ash); volatile constituent: 3.0 mass %; viscosity (4 mass %; 20° C.):  $5.4\pm0.4$  CPS] (all trade names, manufactured by Kuraray Co., Ltd.), and the like.

The above values were measured in the manner described in JIS K-6726-1977.

With respect to modified polyvinyl alcohols, those described in Koichi Nagano, et al., "Poval", Kobunshi Kankokai, Inc. are useful. The modified polyvinyl alcohols include polyvinyl alcohols modified by cations, anions, —SH compounds, alkylthio compounds, or silanols.

Examples of such modified polyvinyl alcohols (modified PVA) include C polymers such as C-118, C-318, C-318-2A, and C-506 (all being trade names of Kuraray Co., Ltd.); HL polymers such as HL-12E and HL-1203 (all being trade names of Kuraray Co., Ltd.); HM polymers such as HM-03 and HM-N-03 (all being trade names of Kuraray Co., Ltd.); K polymers such as KL-118, KL-318, KL-506, KM-118T, and KM-618 (all being trade names of Kuraray Co., Ltd.); M polymers such as M-115 (a trade name of Kuraray Co., Ltd.); MP polymers such as MP-102, MP-202, and MP-203 (all being trade names of Kuraray Co., Ltd.); MPK polymers such as MPK-1, MPK-2, MPK-3, MPK-4, MPK-5, and MPK-6 (all being trade names of Kuraray Co., Ltd.); R polymers such

as R-1130, R-2105, and R-2130 (all being trade names of Kuraray Co., Ltd.); and V polymers such as V-2250 (a trade name of Kuraray Co., Ltd.).

The viscosity of polyvinyl alcohol can be adjusted or stabilized by adding a trace amount of a solvent or an inorganic salt to an aqueous solution of polyvinyl alcohol, and there can be employed compounds described in the aforementioned reference "Poval", Koichi Nagano et al., published by Kobunshi Kankokai, pp. 144-154. For example, a coated-surface quality can be improved by an addition of boric acid, and the addition of boric acid is preferable. The amount of boric acid added is preferably 0.01 to 40 mass % with respect to polyvinyl alcohol.

Preferred binders are transparent or semitransparent, and generally colorless. Examples include natural resins, polymers and copolymers; synthetic resins, polymers, and copolymers; and other media that form films: for example, rubbers, polyvinyl alcohols, hydroxyethyl celluloses, cellulose acetates, cellulose acetate butylates, polyvinylpyrrolidones, starches, polyacrylic acids, polymethyl methacrylates, polyvinyl chlorides, polymethacrylic acids, styrene/maleic acid anhydride copolymers, styrene/acrylonitrile copolymers, styrene/butadiene copolymers, polyvinylacetals (e.g., polyvinylformals and polyvinylbutyral), polyesters, polyurethanes, phenoxy resins, polyvinylidene chlorides, polyepoxides, polycarbonates, polyvinyl acetates, polyolefins, cellulose esters, and polyamides. These media are water-soluble.

In the present invention, preferred water-soluble polymers are polyvinyl alcohols and gelatin, with gelatin being most preferred.

The amount of the water-soluble polymer added to the receptor layer is preferably from 1 to 25% by mass, more preferably from 1 to 10% by mass based on the entire mass of the receptor layer.

<Hardener>

As a crosslinking agent, a hardener (hardening agent) may be added in coating layers (e.g., the receptor layer, the heat insulation layer, the undercoat layer) of the image-receiving sheet.

Preferred examples of the hardener that can be used in the present invention include H-1, 4, 6, 8, and 14 in JP-A-1-214845 in page 17; compounds (H-1 to H-54) represented by one of the formulae (VII) to (XII) in U.S. Pat. No. 4,618,573, columns 13 to 23; compounds (H-1 to H-76) represented by the formula (6) in JP-A-2-214852, page 8, the lower right (particularly, H-14); and compounds described in Claim 1 in U.S. Pat. No. 3,325,287. Examples of the hardening agent include hardening agents described, for example, in U.S. Pat. No. 4,678,739, column 41, U.S. Pat. No. 4,791,042, JP-A-59-116655, JP-A-62-245261, JP-A-61-18942, and JP-A-4-218044. More specifically, an aldehyde-series hardening agent (formaldehyde, etc.), an aziridine-series hardening agent, an epoxy-series hardening agent, a vinyl sulfone-series hardening agent (N,N'-ethylene-bis(vinylsulfonylacetamido) ethane, etc.), an N-methylol-series hardening agent (dimethylol urea, etc.), a boric acid, a metaboric acid, or a polymer hardening agent (compounds described, for example, in JP-A-62-234157), can be mentioned.

Preferred examples of the hardener include a vinylsulfone-series hardener and chlorotriazines.

More preferable hardeners in the present invention are compounds represented by the following Formula (B) or (C).



Formula (B)



Formula (C)

In formulae (B) and (C), X represents a halogen atom, L represents an organic linking group having n-valency. When the compound represented by formula (B) or (C) is a low-molecular compound, n denotes an integer from 1 to 4. When the compound represented by formula (B) or (C) is a high-molecular (polymer) compound, L represents an organic linking group containing a polymer chain and n denotes an integer ranging from 10 to 1,000.

In the Formulae (B) and (C), X is preferably a chlorine atom or a bromine atom, and further preferably a bromine atom. n is an integer from 1 to 4, preferably an integer from 2 to 4, more preferably 2 or 3 and most preferably 2.

L represents an organic group having n-valency, and preferably an aliphatic hydrocarbon group, an aromatic hydrocarbon group or a heterocyclic group, provided that these groups may be combined through an ether bond, ester bond, amide bond, sulfonamide bond, urea bond, urethane bond or the like. Also, each of these groups may be further substituted. Examples of the substituent include a halogen atom, alkyl group, aryl group, heterocyclic group, hydroxyl group, alkoxy group, aryloxy group, alkylthio group, arylthio group, acyloxy group, alkoxy carbonyl group, carbamoyloxy group, acyl group, acyloxy group, acylamino group, sulfonamide group, carbamoyl group, sulfamoyl group, sulfonyl group, phosphoryl group, carboxyl group and sulfo group. Among these groups, a halogen atom, alkyl group, hydroxy group, alkoxy group, aryloxy group and acyloxy group are preferable.

Specific examples of the vinylsulfone-series hardener include, though not limited to, the following compounds (VS-1) to (VS-27).



-continued

(VS-12)



## 19

-continued

(VS-25)



These hardeners may be obtained with reference to the method described in, for example, the specification of U.S. Pat. No. 4,173,481.

Furthermore, as the chlorotriazine-series hardener, a 1,3,5-triazine compound in which at least one of the 2-position, 4-position and 6-position of the triazine ring in the compound is substituted with a chlorine atom, is preferable. A 1,3,5-triazine compound in which two or three of the 2-position, 4-position and 6-position of the triazine ring each are substituted with a chlorine atom, is more preferable. Alternatively, use may be made of a 1,3,5-triazine compound in which at least one of the 2-position, 4-position and 6-position of the triazine ring is substituted with a chlorine atom, and the remainder position(s) is/are substituted with a group(s) or atom(s) other than a chlorine atom. Examples of these other groups include a hydrogen atom, bromine atom, fluorine atom, iodine atom, alkyl group, alkenyl group, alkynyl group, cycloalkyl group, cycloalkenyl group, aryl group, heterocyclic group, hydroxy group, nitro group, cyano group, amino group, hydroxylamino group, alkylamino group, arylamino group, heterocyclic amino group, acylamino group, sulfonamide group, carbamoyl group, sulfamoyl group, sulfo group, carboxyl group, alkoxy group, alkenoxy group, aryloxy group, heterocyclic oxy group, acyl group, acyloxy group, alkyl- or aryl-sulfonyl group, alkyl- or aryl-sulfinyl group, alkyl- or aryl-sulfonyloxy group, mercapto group, alkylthio group, alkenylthio group, arylthio group, heterocyclic thio group and alkyloxy- or aryloxy-carbonyl group.

Specific examples of the chlorotriazine-series hardener include, though not limited to, 4,6-dichloro-2-hydroxy-1,3,5-triazine or its Na salt, 2-chloro-4,6-diphenoxymethyltriazine, 2-chloro-4,6-bis[2,4,6-trimethylphenoxy]triazine, 2-chloro-4,6-diglycidoxo-1,3,5-triazine, 2-chloro-4-(n-butoxy)-6-glycidoxo-1,3,5-triazine, 2-chloro-4-(2,4,6-trimethylphenoxy)-6-glycidoxo-1,3,5-triazine, 2-chloro-4-(2-chloroethoxy)-6-(2,4,6-trimethylphenoxy)-1,3,5-triazine, 2-chloro-4-(2-bromoethoxy)-6-(2,4,6-trimethylphenoxy)-1,3,5-triazine, 2-chloro-4-(2-di-n-butylphosphateethoxy)-6-(2,4,6-trimethylphenoxy)-1,3,5-triazine and 2-chloro-4-(2-di-n-butylphosphateethoxy)-6-(2,6-xylenoxy)-1,3,5-triazine.

Such a compound is easily produced by reacting cyanur chloride (namely, 2,4,6-trichlorotriazine) with, for example, a hydroxy compound, thio compound or amino compound corresponding to the substituent on the heterocycle.

These hardeners are preferably used in an amount of 0.001 to 1 g, and further preferably 0.005 to 0.5 g, per 1 g of the water-soluble polymer.

&lt;Emulsion&gt;

An emulsion is preferably incorporated in the receptor layer of the heat-sensitive transfer image-receiving sheet of

## 20

the present invention. The following is a detailed explanation of the emulsion that is preferably used in the present invention.

Hydrophobic additives, such as a lubricant, an antioxidant, and the like, can be introduced into a layer of the image-receiving sheet (e.g. the receptor layer, the heat insulation layer, the undercoat layer), by using a known method described in U.S. Pat. No. 2,322,027, or the like. In this case, a high-boiling organic solvent, as described in U.S. Pat. No. 4,555,470, U.S. Pat. No. 4,536,466, U.S. Pat. No. 4,536,467, U.S. Pat. No. 4,587,206, U.S. Pat. No. 4,555,476 and U.S. Pat. No. 4,599,296, JP-B-3-62256, and the like, may be used singly or in combination with a low-boiling organic solvent having a boiling point of 50 to 160°C., according to the need. 15 Also, these lubricants, antioxidants, and high-boiling organic solvents may be respectively used in combination of two or more.

As the antioxidant (hereinafter, also referred to as a radical trapper in this specification), a compound represented by any 20 one of the following formulae (E-1) to (E-3) is preferably used.

Formula (E-1)



Formula (E-2)



Formula (E-3)



R<sub>41</sub> represents an aliphatic group, an aryl group, a heterocyclic group, an acyl group, an aliphatic oxycarbonyl group, an aryloxycarbonyl group, an aliphatic sulfonyl group, an arylsulfonyl group, a phosphoryl group, or a group —Si(P<sub>47</sub>)(R<sub>48</sub>)(P<sub>49</sub>) in which R<sub>47</sub>, R<sub>48</sub> and R<sub>49</sub> each independently represent an aliphatic group, an aryl group, an aliphatic oxy group, or an aryloxy group. R<sub>42</sub> to R<sub>46</sub> each independently represent a hydrogen atom, or a substituent. Examples of the substituent include a halogen atom, aliphatic group (including an alkyl group, alkenyl group, alkynyl group, cycloalkyl group, and cycloalkenyl group), aryl group, heterocyclic group, hydroxy group, mercapto group, aliphaticoxyl group,

**21**

aryloxy group, heterocyclic oxy group, aliphaticthio group, arylthio group, heterocyclic thio group, amino group, aliphaticamino group, arylamino group, heterocyclic amino group, acylamino group, sulfonamide group, cyano group, nitro group, carbamoyl group, sulfamoyl group, acyl group, aliphatic oxycarbonyl group, and aryloxycarbonyl group. R<sub>a1</sub>, R<sub>a2</sub>, R<sub>a3</sub>, and R<sub>a4</sub> each independently represent a hydrogen atom, or an aliphatic group (for example, methyl, ethyl). 5

With respect to the compounds represented by any one of the Formulae (E-1) to (E-3), the groups that are preferred from the viewpoint of the effect to be obtained by the present invention, are explained below. 10

In the Formulae (E-1) to (E-3), it is preferred that R<sub>a1</sub> represents an aliphatic group, an acyl group, an aliphatic oxycarbonyl group, an aryloxycarbonyl group, or a phosphoryl group, and R<sub>a2</sub>, R<sub>a3</sub>, R<sub>a5</sub>, and R<sub>a6</sub> each independently represent a hydrogen atom, an aliphatic group, an aliphatic oxy group, or an acylamino group. It is more preferred that R<sub>a1</sub> represents an aliphatic group, and R<sub>a2</sub>, R<sub>a3</sub>, R<sub>a5</sub> and R<sub>a6</sub> independently represent a hydrogen atom or an aliphatic group. 15 20

Preferable specific examples of the compounds represented by any one of the Formulae (E-1) to (E-3) are shown below, but the present invention is not limited to these compounds. 25



EB-1

30



EB-2

35



EB-3

45



EB-4

50



55



65

**22**

-continued

EB-5



EB-6



EB-7



EB-8



EB-9



EB-10



23

-continued



A content of the antioxidant is preferably from 1.0 to 7.0 mass %, more preferably from 2.5 to 5.0 mass %, based on a solid content in the latex polymer.

As the lubricant, solid waxes such as polyethylene wax, amide wax and Teflon (registered trademark) powder; silicone oil, phosphate-series compounds, fluorine-based surfactants, silicone-based surfactants and others including releasing agents known in the technical fields concerned may be used. Fluorine-series compounds typified by fluorine-based surfactants, silicone-based surfactants and silicone-series compounds such as silicone oil and/or its hardened products are preferably used. A content of the lubricant is preferably from 1.0 to 10.0 mass %, more preferably from 1.5 to 2.5 mass %, based on a solid content in the latex polymer.

As the silicone oil as the lubricant, straight silicone oil and modified silicone oil or their hardened products may be used.

Examples of the straight silicone oil include dimethylsilicone oil, methylphenylsilicone oil and methyl hydrogen silicone oil. Examples of the dimethylsilicone oil include KF96-10, KF96-100, KF96-1000, KF96H1-10000, KF96H-12500 and KF96H-100000 (all of these names are trade names, manufactured by Shin-Etsu Chemical Co., Ltd.). Examples of the methylphenylsilicone oil include KF50-100, KF54 and KF56 (all of these names are trade names, manufactured by Shin-Etsu Chemical Co., Ltd.).

The modified silicone oil may be classified into reactive silicone oils and non-reactive silicone oils. Examples of the reactive silicone oils include amino-modified, epoxy-modified, carboxyl-modified, hydroxy-modified, methacryl-modified, mercapto-modified, phenol-modified or one-terminal reactive/hetero-functional group-modified silicone oils. Examples of the amino-modified silicone oil include KF-393, KF-857, KF-858, X-22-3680, X-22-3801C, KF-8010, X-22-161A and KF-8012 (all of these names are trade names, manufactured by Shin-Etsu Chemical Co., Ltd.). Examples of the epoxy-modified silicone oil include KF-100T, KF-101, KF-60-164, KF-103, X-22-343 and X-22-3000T (all of these names are trade names, manufactured by Shin-Etsu Chemical Co., Ltd.). Examples of the carboxyl-modified silicone oil include X-22-162C (trade name, manufactured by Shin-Etsu Chemical Co., Ltd.). Examples of the hydroxy-modified silicone oil include X-22-160AS, KF-6001, KF-6002, KF-6003, X-22-170DX, X-22-176DX, X-22-176D and X-22-176DF (all of these names are trade names, manufactured by Shin-Etsu Chemical Co., Ltd.). Examples of the methacryl-modified silicone oil include X-22-164A, X-22-164C, X-24-8201, X-22-174D and X-22-2426 (all of these names are trade names, manufactured by Shin-Etsu Chemical Co., Ltd.).

Reactive silicone oils may be hardened upon use, and may be classified into a reaction-curable type, photocurable type, catalyst-curable type, and the like. Among these types, silicone oil that is the reaction-curable type is particularly preferable. As the reaction-curable type silicone oil, products obtained by reacting an amino-modified silicone oil with an epoxy-modified silicone oil and then by curing are preferable. Also, examples of the catalyst-curable type or photocurable

EB-11

24

type silicone oil include KS-705F-PS, KS-705F-PS-1 and KS-770-PL-3 (all of these names are trade names, catalyst-curable silicone oils, manufactured by Shin-Etsu Chemical Co., Ltd.) and KS-720 and KS-774-PL-3 (all of these names are trade names, photocurable silicone oils, manufactured by Shin-Etsu Chemical Co., Ltd.). The addition amount of the curable type silicone oil is preferably 0.5 to 30% by mass based on the resin constituting the receptor layer. The releasing agent is used preferably in an amount of 2 to 4% by mass and further preferably 2 to 3% by mass based on 100 parts by mass of the polyester resin. If the amount is too small, the releasability cannot be secured without fail, whereas if the amount is excessive, a protective layer is not transferred to the image-receiving sheet resultantly.

Examples of the non-reactive silicone oil include polyether-modified, methylstyryl-modified, alkyl-modified, higher fatty acid ester-modified, hydrophilic special-modified, higher alkoxy-modified or fluorine-modified silicone oils. Examples of the polyether-modified silicone oil include KF-6012 (trade name, manufactured by Shin-Etsu Chemical Co., Ltd.) and examples of the methylstyryl-modified silicone oil include 24-510 and KF41-410 (all of these names are trade names, manufactured by Shin-Etsu Chemical Co., Ltd.). Modified silicones represented by any one of the following Formulae 1 to 3 may also be used.

Formula 1



In the Formula 1, R represents a hydrogen atom or a straight-chain or branched alkyl group which may be substituted with an aryl or cycloalkyl group. m and n respectively denote an integer of 2,000 or less, and a and b respectively denote an integer of 30 or less.

Formula 2



In the Formula 2, R represents a hydrogen atom or a straight-chain or branched alkyl group which may be substituted with an aryl or cycloalkyl group. m denotes an integer of 2,000 or less, and a and b respectively denote an integer of 30 or less.



In the Formula 3, R represents a hydrogen atom or a straight-chain or branched alkyl group which may be substituted with an aryl or cycloalkyl group. m and n respectively denote an integer of 2,000 or less, and a and b respectively denote an integer of 30 or less. R<sup>1</sup> represents a single bond or a divalent linking group, E represents an ethylene group which may be further substituted, and P represents a propylene group which may be further substituted.

Silicone oils such as those mentioned above are described in "SILICONE HANDBOOK" (The Nikkan Kogyo Shim bun, Ltd.) and the technologies described in each publication of JP-A-8-108636 and JP-A-2002-264543 may be preferably used as the technologies to cure the curable type silicone oils.

Examples of the high-boiling organic solvent include phthalates (e.g., dibutyl phthalate, dioctyl phthalate, di-2-ethylhexyl phthalate), phosphates or phosphonates (e.g., triphenyl phosphate, tricresyl phosphate, tri-2-ethylhexyl phosphate), fatty acid esters (e.g., di-2-ethylhexyl succinate, tributyl citrate), benzoates (e.g., 2-ethylhexyl benzoate, dodecyl benzoate), amides (e.g., N,N-diethyldodecane amide, N,N-dimethylolein amide), alcohols or phenols (e.g., iso-stearyl alcohol, 2,4-di-tert-amyl phenol), anilines (e.g., N,N-dibutyl-2-butoxy-5-tert-octylaniline), chlorinated paraffins, hydrocarbons (e.g., dodecyl benzene, diisopropyl naphthalene), and carboxylic acids (e.g., 2-(2,4-di-tert-amyl phenoxy)butyrate).

Preferably the compounds shown below are used.

Formula 3

5

10

15

-continued

(Solv-7)



(Solv-8)

(Solv-9)

Further, the high-boiling organic solvent may be used in combination with, as an auxiliary solvent, an organic solvent having a boiling point of 30° C. or more and 160° C. or less, such as ethyl acetate, butyl acetate, methyl ethyl ketone, cyclohexanone, methylcellosolve acetate, or the like. The high-boiling organic solvent is used in an amount of generally 1 to 10 g, preferably 5 g or less, and more preferably 1 to 0.1 g, per 1 g of the hydrophobic additives to be used. The amount is also preferably 1 ml or less, more preferably 0.5 ml or less, and particularly preferably 0.3 ml or less, per 1 g of the binder.

A dispersion method that uses a polymer, as described in JP-B-51-39853 and JP-A-51-59943, and a method wherein the addition is made with them in the form of a dispersion of fine particles, as described in, for example, JP-A-62-30242, can also be used. In the case of a compound that is substantially insoluble in water, other than the above methods, a method can be used wherein the compound is dispersed and contained in the form of fine particles in a binder.

When the hydrophobic compound is dispersed in a hydrophilic colloid, various surfactants may be used. For example, those listed as examples of the surfactant in JP-A-59-157636, page (37) to page (38) may be used. It is also possible to use phosphates-based surfactants described in JP-A-7-56267, JP-A-7-228589, and West German Patent Application Laid-Open (OLS) No. 1,932,299A.

## &lt;Ultraviolet Absorber&gt;

Also, in the present invention, in order to improve light resistance, an ultraviolet absorber may be added to the receptor layer. In this case, when this ultraviolet absorber is made to have a higher molecular weight, it can be secured to the receptor layer so that it can be prevented, for instance, from being diffused into the ink sheet and from being sublimated and vaporized by heating.

As the ultraviolet absorber, compounds having various ultraviolet absorber skeletons, which are widely used in the field of information recording, may be used. Specific examples of the ultraviolet absorber may include compounds having a 2-hydroxybenzotriazole type ultraviolet absorber

skeleton, 2-hydroxybenzotriazine type ultraviolet absorber skeleton, or 2-hydroxybenzophenone type ultraviolet absorber skeleton. Compounds having a benzotriazole-type or triazine-type skeleton are preferable from the viewpoint of ultraviolet absorbing ability (absorption coefficient) and stability,

and compounds having a benzotriazole-type or benzophenone-type skeleton are preferable from the viewpoint of obtaining a higher-molecular weight and using in a form of a latex. Specifically, ultraviolet absorbers described in, for example, JP-A-2004-361936 may be used.

The ultraviolet absorber preferably absorbs light at wavelengths in the ultraviolet region, and the absorption edge of the absorption of the ultraviolet absorber is preferably out of



(Solv-1)

(Solv-2)



(Solv-3)



(Solv-4)



(Solv-5)



(Solv-6)



the visible region. Specifically, when it is added to the receptor layer to form a heat-sensitive transfer image-receiving sheet, the heat-sensitive transfer image-receiving sheet has a reflection density of, preferably, Abs 0.5 or more at 370 nm, and more preferably Abs 0.5 or more at 380 nm. Also, the heat-sensitive transfer image-receiving sheet has a reflection density of, preferably, Abs 0.1 or less at 400 nm. If the reflection density at a wavelength range exceeding 400 nm is high, it is not preferable because an image is made yellowish.

In the present invention, the ultraviolet absorber is preferably made to have a higher molecular weight. The ultraviolet absorber has a mass average molecular weight of preferably 10,000 or more, and more preferably 100,000 or more. As a means of obtaining a higher-molecular weight ultraviolet absorber, it is preferable to graft an ultraviolet absorber on a polymer. The polymer as the principal chain preferably has a polymer skeleton less capable of being dyed than the receptor polymer to be used together. Also, when the polymer is used to form a film, the film preferably has sufficient film strength. The graft ratio of the ultraviolet absorber to the polymer principal chain is preferably 5 to 20% by mass and more preferably 8 to 15% by mass.

Also, it is more preferable that the ultraviolet-absorber-grafted polymer is made to be used in a form of a latex. When the polymer is made to be used in a form of a latex, an aqueous dispersion-system coating solution may be used in application and coating to form the receptor layer, and this enables reduction of production cost. As a method of making the latex polymer (or making the polymer latex-wise), a method described in, for example, Japanese Patent No. 3450339 may be used. As the ultraviolet absorber to be used in a form of a latex, the following commercially available ultraviolet absorbers may be used which include ULS-700, ULS-1700, ULS-1383MA, ULS-1635MH, XL-7016, ULS-933LP, and ULS-935LH, manufactured by Ipposha Oil Industries Co., Ltd.; and New Coat UVA-1025W, New Coat UVA-204W, and New Coat UVA-4512M, manufactured by Shin-Nakamura Chemical Co., Ltd. (all of these names are trade names).

In the case of using an ultraviolet-absorber-grafted polymer in a form of a latex, it may be mixed with a latex of the receptor polymer capable of being dyed, and the resulting mixture is coated. By doing so, a receptor layer, in which the ultraviolet absorber is homogeneously dispersed, can be formed.

The addition amount of the ultraviolet-absorber-grafted polymer or its latex is preferably 5 to 50 parts by mass, and more preferably 10 to 30 parts by mass, to 100 parts by mass of the receptor latex polymer capable of being dyed to be used to form the receptor layer.

<Releasing Agent>

Also, a releasing agent may be compounded in the receptor layer, in order to prevent thermal fusion with the heat-sensitive transfer sheet when an image is formed. As the releasing agent, a silicone oil, a phosphate-based plasticizer, a fluorine-series compound, or various wax dispersions may be used, and the silicone oil and the wax dispersions are particularly preferably used.

As the silicone oil, modified silicone oil, such as epoxy-modified, alkyl-modified, amino-modified, carboxyl-modified, alcohol-modified, fluorine-modified, alkyl aralkyl poly-ether-modified, epoxy/polyether-modified, or polyether-modified silicone oil, is preferably used. Among these, a reaction product between vinyl-modified silicone oil and hydrogen-modified silicone oil is preferable. The amount of the releasing agent is preferably 0.2 to 30 parts by mass, per 100 parts by mass of the receptor polymer.

As the wax dispersions, known dispersions may be used. In the present invention, "wax" means an organic compound having an alkyl chain which is in a solid or semisolid state at room temperature (according to the definition given in *Kaitei Wax no Seishitsu to Oyo* (Revised edition, Properties and Applications of Wax), Sawai Shobo (1989)). Preferable examples of the organic compound include candelilla wax, carnauba wax, rice wax, haze wax, montan wax, ozokerite, paraffin wax, microcrystalline wax, petrolatum, Fischer-  
10 Tropsch wax, polyethylene wax, montan wax derivatives, paraffin wax derivatives, microcrystalline wax derivatives, hydrogenated ricinus, hydrogenated ricinus derivatives, 12-hydroxystearic acid, stearic acid amide, phthalic anhydride imide, chlorinated hydrocarbons, and other mixed  
15 waxes. Of these waxes, carnauba wax, montan wax and derivatives thereof, paraffin wax and derivatives thereof, microcrystalline wax and derivatives thereof, polyethylene wax and stearic acid amide are preferred; carnauba wax, montan wax and derivatives thereof, microcrystalline wax and stearic acid amide are more preferred; and montan wax, montan wax derivatives and microcrystalline wax are further preferred.

These waxes are selected from waxes having melting points of generally 25° C. to 120° C., preferably 40° C. to 100° C., more preferably 60° C. to 90° C.

The wax is preferably in a state of being dispersed in water, more preferably in the form of fine particles. Dispersing waxes in water and forming waxes into fine particles can be performed using the methods as described in "Kaitei Wax no Seishitsu to Oyo (Revised version, Properties and Applications of Wax)", Sawai Shobo (1989).

The addition amount of wax is preferably from 0.5 to 30% by mass, more preferably from 1 to 20% by mass, and further preferably from 1.5 to 15% by mass, of the amount of total solid content in the receptor layer.

The amount of the receptor layer to be applied is preferably 0.5 to 10 g/m<sup>2</sup> (solid basis, hereinafter, the amount to be applied in the present specification means a value on solid basis unless otherwise noted), more preferably 1 to 8 g/m<sup>2</sup>, and further preferably 2 to 7 g/m<sup>2</sup>. The film thickness of the receptor layer is preferably 1 to 20 µm.

In addition, when the receptor layer has both the upper layer and the lower layer, each of the ratio of coating amount and the ratio of film thickness of the upper layer and the lower layer is not particularly limited. The ratio of the coating amount of the upper layer to that of the lower layer is preferably 5:100 to 500:100, more preferably 10:100 to 200:100, and further more preferably 20:100 to 150:100, and the ratio of the film thickness of the upper layer to that of the lower layer is preferably 5:100 to 500:100, more preferably 10:100 to 200:100, and further more preferably 20:100 to 150:100. (Heat Insulation Layer)

A heat insulation layer serves to protect the support from heat when a thermal head or the like is used to carry out a transfer operation under heating. Also, because the heat insulation layer generally has proper cushion characteristics, a heat-sensitive transfer image-receiving sheet having high printing sensitivity can be obtained even in the case of using paper as a substrate (support). The heat insulation layer may be a single layer, or multi-layers. The heat insulation layer is generally arranged at a nearer location to the support than the receptor layer.

In the image-receiving sheet of the present invention, the heat insulation layer contains at least one kind of hollow latex polymer particles and at least one water-soluble polymer.

The hollow polymer particles in the present invention are polymer particles having independent pores inside of the

particles. Examples of the hollow polymer particles include (1) non-foaming type hollow particles obtained in the following manner: a dispersion medium such as water is contained inside of a capsule wall formed of a polystyrene, acryl resin, or styrene/acryl resin and, after a coating solution is applied and dried, the dispersion medium in the particles is vaporized out of the particles, with the result that the inside of each particle forms a hollow; (2) foaming type microballoons obtained in the following manner: a low-boiling point liquid such as butane and pentane is encapsulated in a resin constituted of any one of polyvinylidene chloride, polyacrylonitrile, polyacrylic acid and polyacrylate, and their mixture or polymer, and after the resin coating material is applied, it is heated to expand the low-boiling point liquid inside of the particles whereby the inside of each particle is made to be hollow; and (3) microballoons obtained by foaming the above (2) under heating in advance, to make hollow polymer particles.

The hollow latex polymer particles for use in the present invention are a latex of the above-described hollow polymers particles. Hereinafter, the hollow latex polymer particles are also referred to as hollow polymer particles.

The particle size of the hollow polymer particles is preferably 0.1 to 20  $\mu\text{m}$ , more preferably 0.1 to 2  $\mu\text{m}$ , further preferably 0.1 to 1  $\mu\text{m}$ , particularly preferably 0.2 to 0.8  $\mu\text{m}$ . It is because an excessively small size may lead to decrease of the void ratio (hollow ratio) of the particles, prohibiting desirable heat-insulating efficiency, while an excessively large size in relation to the thickness of the heat insulation layer may result in problems for preparation of smooth surface and cause coating troubles due to the bulky particles.

These hollow polymer particles preferably have a hollow ratio of about 20 to 70%, more preferably 20 to 50%. With too small hollow ratio, it cannot give a sufficient heat-insulating efficiency, while with an excessively large hollow ratio for the hollow particles that have the above-described preferable particle diameter, imperfect hollow particles increase prohibiting sufficient film strength.

The "hollow ratio" of the hollow polymer particles as referred to here is a value P calculated according to the Formula (a), based on the transmission image photographed by a transmission micrograph of hollow particles.

$$P = \left\{ \frac{1}{n} \times \sum_{i=1}^n (Rai / Rbi)^3 \right\} \times 100 (\%)$$

Formula (a)

In formula (a), Rai represents a circle-equivalent diameter of the inner periphery (which shows the periphery of a hollow portion), among two peripheries constituting an image of a specific particle i; Rbi represents a circle-equivalent diameter of the outer periphery (which shows the outer shape of a particle in interest), among the two peripheries constituting the image of the specific particle i; and n is the number of measured particles, and n is generally 300 or more. Herein, the term "circle-equivalent diameter" means the diameter of a circle having an area equivalent to the (projected) area that the hollow portion's periphery or the particle's outer shape has.

The glass transition temperature ( $T_g$ ) of the hollow polymer particles is preferably 70°C. or more and more preferably 100°C. or more. These hollow polymer particles may be used in combinations of two or more.

Such hollow polymer particles are commercially available. Specific examples of the above (1) include Rohpake 1055 manufactured by Rohm and Haas Co.; Boncoat PP-1000 manufactured by Dainippon Ink and Chemicals, Incorpor-

rated; SX866(B) manufactured by JSR Corporation; and Nip-pol MH15055 manufactured by Nippon Zeon (all of these product names are trade names). Specific examples of the above (2) include F-30 and F-50 manufactured by Matsumoto Yushi-Seiyaku Co., Ltd. (all of these product names are trade names). Specific examples of the above (3) include F-30E manufactured by Matsumoto Yushi-Seiyaku Co., Ltd., and Expance 461DE, 551DE and 551DE20 manufactured by Nippon Ferrite (all of these product names are trade names). 10 Among these, the hollow polymer particles of the above (1) may be preferably used.

At least one water-soluble polymer, namely a water-dispersible resin or water-soluble type resin, is used as a binder, in the heat insulation layer containing the hollow polymer particles. 15 As the binder resin that can be used in the present invention, known resins such as an acryl resin, styrene/acryl copolymer, polystyrene resin, polyvinyl alcohol resin, vinyl acetate resin, ethylene/vinyl acetate copolymer, vinyl chloride/vinyl acetate copolymer, styrene/butadiene copolymer, 20 polyvinylidene chloride resin, cellulose derivative, casein, starch, and gelatin may be used. Also, these resins may be used either singly or as mixtures.

The solid content of the hollow polymer particles in the heat insulation layer preferably falls in a range from 5 to 2,000 25 parts by mass, more preferably 5 to 1000 parts by mass, and further preferably 5 to 400 parts by mass, assuming that the solid content of the binder resin be 100 parts by mass. Also, the ratio by mass of the solid content of the hollow polymer particles in the coating solution is preferably 1 to 70% by 30 mass and more preferably 10 to 40% by mass. If the ratio of the hollow polymer particles is excessively low, sufficient heat insulation cannot be obtained, whereas if the ratio of the hollow polymer particles is excessively large, the adhesion between the hollow polymer particles is reduced, and thereby 35 sufficient film strength cannot be obtained, causing deterioration in abrasion resistance.

The heat insulation layer of the heat-sensitive transfer image-receiving sheet of the present invention is preferably 40 free of any resins that are not resistant to an organic solvent, except for the hollow polymer particles. Incorporation of the resin that is not resistant to an organic solvent (resin having a dye-dyeing affinity) in the heat insulation layer is not preferable in view of increase in loss of image definition after image 45 transfer. It is assumed that the color-edge definition loss increases by the reason that owing to the presence of both the resin having a dye-dyeing affinity and the hollow polymer particles in the heat insulation layer, a transferred dye that has dyed the receptor layer migrates through the heat insulation layer adjacent thereto with the lapse of time.

50 Herein, the term "the resin that is not resistant to an organic solvent" means a resin having a solubility in an organic solvent (e.g., methyl ethyl ketone, ethyl acetate, benzene, toluene, xylene) of 1 mass % or more, preferably 0.5 mass % or more. For example, the above-mentioned latex polymer is 55 included in the category of "the resin that is not resistant to an organic solvent".

The water-soluble polymer used in the heat-insulating layer is preferably any of the water-soluble polymers described above as those used in the receptor layer. Preferable 60 compounds of the water-soluble polymer are the same as mentioned above.

An amount of the water-soluble polymer to be added in the heat insulation layer is preferably from 1 to 75 mass %, more 65 preferably from 1 to 50 mass % to the entire heat insulation layer.

The heat insulation layer preferably contains a gelatin. The amount of the gelatin in the coating solution for the heat

## 31

insulation layer is preferably 0.5 to 14% by mass, and particularly preferably 1 to 6% by mass. Also, the coating amount of the above hollow polymer particles in the heat insulation layer is preferably 1 to 100 g/m<sup>2</sup>, and more preferably 5 to 20 g/m<sup>2</sup>.

The heat insulation layer preferably contains a crosslinking agent (compound capable of crosslinking a water-soluble polymer). A part or all of the water-soluble polymer that is contained in the heat insulation layer has been preferably cross-linked with the crosslinking agent. Preferable compounds as well as a preferable amount of the crosslinking agent to be used are the same as mentioned above.

A preferred ratio of a cross-linked water-soluble polymer in the heat insulation layer varies depending on the kind of the crosslinking agent, but the water-soluble polymer in the heat insulation layer is crosslinked by preferably 0.1 to 20 mass %, more preferably 1 to 10 mass %, based on the entire water-soluble polymer.

A thickness of the heat insulation layer containing the hollow polymer particles is preferably from 5 to 50 µm, more preferably from 5 to 40 µm.

A void ratio (porosity ratio) of the heat insulation layer, which is calculated from the thickness of the heat insulation layer containing hollow polymer particles and the solid-matter coating amount of the heat insulation layer including the hollow polymer particles, is preferably 10 to 70% and more preferably 15 to 60%. When the void ratio is too low, sufficient heat insulation property cannot be obtained. When the void ratio is too large, the binding force among hollow polymer particles deteriorates, and thus sufficient film strength cannot be obtained, and abrasion resistance deteriorates.

The void ratio of the heat insulation layer as referred to here is a value V calculated according to the Formula (b) below.

$$V = 1 - L / L \times \sum g_i \cdot d_i$$

Formula (b)

In Formula (b), L represents the thickness of the heat-insulating layer; g<sub>i</sub> represents the coating amount of a particular material i in terms of solid matter for the heat-insulating layer; and d<sub>i</sub> represents the specific density of the particular material i. When d<sub>i</sub> represents the specific density of the hollow polymer particles, d<sub>i</sub> is the specific density of the wall material of hollow polymer particles.

(Undercoat Layer)

An undercoat layer may be formed between the receptor layer and the heat insulation layer. As the undercoat layer, for example, at least one of a white background controlling layer, a charge controlling layer, an adhesive layer, and a primer layer is formed. These layers may be formed in the same manner as those described in, for example, each specification of Japanese Patent Nos. 3585599 and 2925244.

(Support)

In the present invention, a waterproof support is preferably used as the support. The use of the waterproof support makes it possible to prevent the support from absorbing moisture, whereby a fluctuation in the performance of the receptor layer with time can be prevented. As the waterproof support, for example, coated paper or laminate paper may be used.

—Coated Paper—

The coated paper is paper obtained by coating a sheet such as base paper with various resins, rubber latexes, or high-molecular materials, on one side or both sides of the sheet, wherein the coating amount differs depending on its use. Examples of such coated paper include art paper, cast coated paper, and Yankee paper.

It is proper to use a thermoplastic resin as the resin to be applied to the surface(s) of the base paper and the like. As

## 32

such a thermoplastic resin, the following thermoplastic resins (A) to (H) may be exemplified.

(A) Polyolefin resins such as polyethylene resin and polypropylene resin; copolymer resins composed of an olefin such as ethylene or propylene and another vinyl monomer; and acrylic resins.

(B) Thermoplastic resins having an ester linkage: for example, polyester resins obtained by condensation of a dicarboxylic acid component (such a dicarboxylic acid component may be substituted with a sulfonic acid group, a carboxyl group, or the like) and an alcohol component (such an alcohol component may be substituted with a hydroxyl group, or the like); polyacrylate resins or polymethacrylate resins such as polymethylmethacrylate, polybutylmethacrylate, polymethylacrylate, polybutylacrylate, or the like; polycarbonate resins, polyvinyl acetate resins, styrene acrylate resins, styrene-methacrylate copolymer resins, vinyltoluene acrylate resins, or the like.

Concrete examples of them are those described in JP-A-59-101395, JP-A-63-7971, JP-A-63-7972, JP-A-63-7973, and JP-A-60-294862.

Commercially available thermoplastic resins usable herein are, for example, Vylon 290, Vylon 200, Vylon 280, Vylon 300, Vylon 103, Vylon GK-140, and Vylon GK-130 (products of Toyobo Co., Ltd.); Tafton NE-382, Tafton U-5, ATR-2009, and ATR-2010 (products of Kao Corporation); Elitel UE 3500, UE 3210, XA-8153, KZA-7049, and KZA-1449 (products of Unitika Ltd.); and Polyester TP-220 and R-188 (products of The Nippon Synthetic Chemical Industry Co., Ltd.); and thermoplastic resins in the Hyros series from Seiko Chemical Industries Co., Ltd., and the like (all of these names are trade names).

(C) Polyurethane resins, etc.

(D) Polyamide resins, urea resins, etc.

(E) Polysulfone resins, etc.

(F) Polyvinyl chloride resins, polyvinylidene chloride resins, vinyl chloride/vinyl acetate copolymer resins, vinyl chloride/vinyl propionate copolymer resins, etc.

(G) Polyol resins such as polyvinyl butyral; and cellulose resins such as ethyl cellulose resin and cellulose acetate resin.

(H) Polycaprolactone resins, styrene/maleic anhydride resins, polyacrylonitrile resins, polyether resins, epoxy resins, and phenolic resins.

The thermoplastic resins may be used either alone or in combination of two or more.

The thermoplastic resin may contain a whitener, a conductive agent, a filler, a pigment or dye including, for example, titanium oxide, ultramarine blue, and carbon black; or the like, if necessary.

—Laminated Paper—

The laminated paper is a paper which is formed by laminating various kinds of resin, rubber, polymer sheets or films on a sheet such as a base paper or the like. Specific examples of the materials useable for the lamination include polyolefins, polyvinyl chlorides, polyethylene terephthalates, polystyrenes, polymethacrylates, polycarbonates, polyimides, and triacetylcelluloses. These resins may be used alone, or in combination of two or more.

Generally, the polyolefins are prepared by using a low-density polyethylene. However, for improving the thermal resistance of the support, it is preferred to use a polypropylene, a blend of a polypropylene and a polyethylene, a high-density polyethylene, or a blend of a high-density polyethylene and a low-density polyethylene. From the viewpoint of cost and its suitability for the laminate, it is preferred to use the blend of a high-density polyethylene and a low-density polyethylene.

The blend of a high-density polyethylene and a low-density polyethylene is preferably used in a blend ratio (a mass ratio) of 1/9 to 9/1, more preferably 2/8 to 8/2, and most preferably 3/7 to 7/3. When the thermoplastic resin layer is formed on the both surfaces of the support, the back side of the support is preferably formed using, for example, the high-density polyethylene or the blend of a high-density polyethylene and a low-density polyethylene. The molecular weight of the polyethylenes is not particularly limited. Preferably, both of the high-density polyethylene and the low-density polyethylene have a melt index of 1.0 to 40 g/10 minute and a high extrudability.

The sheet or film may be subjected to a treatment to impart white reflection thereto. As a method of such a treatment, for example, a method of incorporating a pigment such as titanium oxide into the sheet or film can be mentioned.

The thickness of the support is preferably from 25  $\mu\text{m}$  to 300  $\mu\text{m}$ , more preferably from 50  $\mu\text{m}$  to 260  $\mu\text{m}$ , and further preferably from 75  $\mu\text{m}$  to 220  $\mu\text{m}$ . The support can have any rigidity according to the purpose. When it is used as a support for electrophotographic image-receiving sheet of photographic image quality, the rigidity thereof is preferably near to that in a support for use in color silver halide photography. (Curling Control Layer)

When the support is exposed as it is, there is the case where the heat-sensitive transfer image-receiving sheet is made to curl by moisture and/or temperature in the environment. It is therefore preferable to form a curling control layer on the backside of the support. The curling control layer not only prevents the image-receiving sheet from curling but also has a water-proof function. For the curling control layer, a polyethylene laminate, a polypropylene laminate or the like is used. Specifically, the curling control layer may be formed in a manner similar to those described in, for example, JP-A-61-110135 and JP-A-6-202295.

(Writing Layer and Charge Controlling Layer)

For the writing layer and the charge control layer, an inorganic oxide colloid, an ionic polymer, or the like may be used. As the antistatic agent, any antistatic agents including cationic antistatic agents such as a quaternary ammonium salt and polyamine derivative, anionic antistatic agents such as alkyl phosphate, and nonionic antistatic agents such as fatty acid ester may be used. Specifically, the writing layer and the charge control layer may be formed in a manner similar to those described in the specification of Japanese Patent No. 3585585.

The method of producing the heat-sensitive transfer image-receiving sheet for use in the present invention is explained below.

The heat-sensitive transfer image-receiving sheet of the present invention can be preferably formed, by applying at least one receptor layer, at least one intermediate layer and at least one heat-insulating layer, on a support, through simultaneous multi-layer coating.

It is known that in the case of producing an image-receiving sheet composed of plural layers having different functions from each other (for example, an air cell layer, a heat insulation layer, an intermediate layer and a receptor layer) on a support, it may be produced by applying each layer successively one by one, or by overlapping the layers each already coated on a support or substrate, as shown in, for example, JP-A-2004-106283, JP-A-2004-181888 and JP-A-2004-345267. It has been known in photographic industries, on the other hand, that productivity can be greatly improved, for example, by providing plural layers through simultaneous multi-layer coating. For example, there are known methods such as the so-called slide coating (slide coating method) and curtain coating (curtain coating method) as described in, for example, U.S. Pat. Nos. 2,761,791, 2,681,234, 3,508,947, 4,457,256 and 3,993,019; JP-A-63-54975, JP-A-61-278848, JP-A-55-86557, JP-A-52-31727, JP-A-55-142565, JP-A-50-

43140, JP-A-63-80872, JP-A-54-54020, JP-A-5-104061, JP-A-5-127305, and JP-B-49-7050; and Edgar B. Gutoff, et al., "Coating and Drying Defects: Troubleshooting Operating Problems", John Wiley & Sons Company, 1995, pp. 101-103.

5 In the present invention, it has been found that the productivity is greatly improved and, at the same time, image defects can be remarkably reduced, by using the above simultaneous multilayer coating for the production of an image-receiving sheet having a multilayer structure.

10 The plural layers in the present invention are structured using resins as its major components. Coating solutions forming each layer are preferably water-dispersible latexes. The solid content by mass of the resin put in a latex state in each layer coating solution is preferably in a range from 5 to 80% and particularly preferably 20 to 60%. The average particle size of the resin contained in the above water-dispersed latex is preferably 5  $\mu\text{m}$  or less and particularly preferably 1  $\mu\text{m}$  or less. The above water-dispersed latex may contain a known additive, such as a surfactant, a dispersant, and a binder resin, according to the need.

15 20 In the present invention, it is preferred that a laminate composed of plural layers be formed on a support and solidified just after the forming, according to the method described in U.S. Pat. No. 2,761,791. For example, in the case of solidifying a multilayer structure by using a resin, it is preferable to raise the temperature immediately after the plural layers are formed on the support. Also, in the case where a binder (e.g., a gelatin) to be gelled at lower temperatures is contained, there is the case where it is preferable to drop the temperature immediately after the plural layers are formed on the support.

25 30 In the present invention, the coating amount of a coating solution per one layer constituting the multilayer is preferably in a range from 1  $\text{g}/\text{m}^2$  to 500  $\text{g}/\text{m}^2$ . The number of layers in the multilayer structure may be arbitrarily selected from a number of 2 or more. The receptor layer is preferably disposed as a layer most apart from the support.

35 40 45 A heat-sensitive transfer sheet (ink sheet) used in combination with the heat-sensitive transfer image-receiving sheet according to the present invention as mentioned above at the time of formation of heat transfer image is preferably a sheet having on a support a dye layer containing a diffusion-transfer dye, and any ink sheet can be used as the sheet. As a means for providing heat energy in the thermal transfer, any of the conventionally known providing means may be used. For example, application of a heat energy of about 5 to 100  $\text{mJ}/\text{mm}^2$  by controlling recording time in a recording device such as a thermal printer (trade name: Video Printer VY-100, manufactured by Hitachi, Ltd.), sufficiently attains the expected result.

50 55 60 Also, the heat-sensitive transfer image-receiving sheet of the present invention may be used in various applications enabling thermal transfer recording, such as heat-sensitive transfer image-receiving sheets in a form of thin sheets (cut sheets) or rolls; cards; and transmittable type manuscript-making sheets, by optionally selecting the type of support.

The present invention can be applied to a printer, a copying machine and the like, each of which uses a heat-sensitive transfer recording system.

65 70 75 The present invention can provide a heat-sensitive transfer image-receiving sheet which gives high-quality images of high densities and, in particular, causes no transfer failure, with utilizing the multilayer coating using aqueous coating solutions which method enables high productivity. Further, the present invention can also provide a heat-sensitive transfer image-receiving sheet excellent in long-term preservability.

According to the present invention, it is possible to provide a heat-sensitive transfer image-receiving sheet which has high sensitivity, and can form a high-quality image high in density and excellent in long-term preservability. Further, it is possible to provide a production method of the heat-sensitive

transfer image-receiving sheet which exhibits high productivity and is excellent in safety and environmental friendliness.

The present invention will be described in more detail based on the following examples, but the invention is not intended to be limited thereto.

### EXAMPLES

In the following Examples, the terms "part" and "%" are values by mass, unless they are indicated differently in particular.

#### (Preparation of Ink Sheet)

A polyester film 6.0  $\mu\text{m}$  in thickness (trade name: Lumiror, manufactured by Toray Industries, Inc.) was used as the substrate film. A heat-resistant slip layer (thickness: 1  $\mu\text{m}$ ) was formed on the back side of the film, and the following yellow, magenta, and cyan compositions were respectively applied as a monochromatic layer (coating amount: 1 g/ $\text{m}^2$  after drying) on the front side.

| Yellow composition                                                                          |                   |
|---------------------------------------------------------------------------------------------|-------------------|
| Dye (trade name: Macrolex Yellow 6G, manufactured by Byer)                                  | 5.5 parts by mass |
| Polyvinylbutyral resin (trade name: ESLEC BX-1, manufactured by Sekisui Chemical Co., Ltd.) | 4.5 parts by mass |
| Methyl ethyl ketone/toluene (1/1, at mass ratio)                                            | 90 parts by mass  |
| Magenta composition                                                                         |                   |
| Magenta dye (trade name: Disperse Red 60)                                                   | 5.5 parts by mass |
| Polyvinylbutyral resin (trade name: ESLEC BX-1, manufactured by Sekisui Chemical Co., Ltd.) | 4.5 parts by mass |
| Methyl ethyl ketone/toluene (1/1, at mass ratio)                                            | 90 parts by mass  |
| Cyan composition                                                                            |                   |
| Cyan dye (Solvent Blue 63)                                                                  | 5.5 parts by mass |
| Polyvinylbutyral resin (trade name: ESLEC BX-1, manufactured by Sekisui Chemical Co., Ltd.) | 4.5 parts by mass |
| Methyl ethyl ketone/toluene (1/1, at mass ratio)                                            | 90 parts by mass  |

#### (Preparation of Image-Receiving Sheet)

#### (Preparation of Support)

A pulp slurry was prepared from 50 parts by mass of hardwood bleach kraft pulp (LBKP) of acacia origin and 50 parts by mass of hardwood bleach kraft pulp (LBKP) of aspen origin, by beating these pulps by means of a disk refiner until Canadian standard freeness reached to 300 ml.

To the pulp slurry thus prepared were added, on a pulp basis, 1.3 mass % of modified cationic starch (CAT0304L, trade name, manufactured by Nippon NSC), 0.15 mass % of anionic polyacrylamide (DA4104, trade name, manufactured by Seiko PMC Corporation), 0.29 mass % of an alkylketene dimer (SIZEPINE K, trade name, manufactured by Arakawa Chemical Industries, Ltd.), 0.29 mass % of epoxidized behenic acid amide, and 0.32 mass % of polyamide polyamine epichlorohydrin (ARAFIX 100, trade name, manufactured by Arakawa Chemical Industries, Ltd.), and thereafter 0.12 mass % of a defoaming agent was further added.

The resulting pulp slurry was made into paper by use of a fourdrinier paper machine. In a process of drying in which the felt side of web was pressed against a drum dryer cylinder via a dryer canvas, the web thus formed was dried under a condition that the tensile strength of the dryer canvas was adjusted to 1.6 kg/cm. Then, each side of the raw paper thus made was coated with 1 g/ $\text{m}^2$  of polyvinyl alcohol (KL-118, trade name, manufactured by Kuraray Co., Ltd.) with a size press, then, dried and further subjected to calendering treatment. Therein, the papermaking was performed so that the

raw paper had a grammage (basis weight) of 157 g/ $\text{m}^2$ , and the raw paper (base paper) having a thickness of 160  $\mu\text{m}$  was obtained.

The wire side (back side) of the base paper obtained was subjected to corona discharge treatment, and thereto a resin composition, in which a high-density polyethylene having an MFR (which stands for a melt flow rate, and hereinafter has the same meaning) of 16.0 g/10 min and a density of 0.96 g/ $\text{cm}^3$  (containing 250 ppm of hydrotalcite (DHT-4A (trade name), manufactured by Kyowa Chemical Industry Co., Ltd.) and 200 ppm of a secondary oxidation inhibitor (tris(2,4-di-t-butylphenyl)phosphite, Irugaphos 168 (trade name), manufactured by Ciba Specialty Chemicals)) and a low-density polyethylene having an MFR of 4.0 g/10 min and a density of 0.93 g/ $\text{cm}^3$  were mixed at a ratio of 75 to 25 by mass, was applied so as to have a thickness of 21 g/ $\text{m}^2$ , by means of a melt extruder, thereby forming a thermoplastic resin layer with a mat surface. (The side to which this thermoplastic resin layer was provided is hereinafter referred to as "back side").

The thermoplastic resin layer at the back side was further subjected to corona discharge treatment, and then coated with a dispersion prepared by dispersing into water a 1:2 mixture (by mass) of aluminum oxide (ALUMINASOL 100, trade name, manufactured by Nissan Chemical Industries, Ltd.) and silicon dioxide (SNOWTEX O, trade name, manufactured by Nissan Chemical Industries, Ltd.), as an antistatic agent, so that the coating had a dry mass of 0.2 g/ $\text{m}^2$ . Subsequently, the front surface (front side) of the base paper was subjected to corona discharge treatment, and then coated with 27 g/ $\text{m}^2$  of a low-density polyethylene having an MFR of 4.0 g/10 min and a density of 0.93 g/ $\text{cm}^3$  and containing 10 mass % of titanium oxide, by means of a melt extruder, thereby forming a thermoplastic resin layer with a specular surface.

### Example 1

#### Preparation of Latex Polymer

#### Synthetic Examples

##### (Synthesis of Emulsion-1)

After the atmosphere in a polymerization vessel equipped with a stirrer, a condenser, a thermometer, and an inlet for introduction of nitrogen gas, was thoroughly replaced with N<sub>2</sub>, 1,150 g of deionized water, 100 g of ethyl acrylate, and 30 g of sodium dodecylbenzenesulfonate were placed in the vessel, the pressure inside the polymerization vessel was reduced, and then 900 parts by mass of vinyl chloride was further placed therein. After the temperature inside the polymerization vessel was raised to 60° C., 50 parts by mass of a 1% aqueous solution of ammonium persulfate was introduced under pressure to initiate polymerization reaction, and the reaction was continued for 16 hours as the inside temperature was kept at 60° C., to attain completion of the polymerization. Thereafter, the reaction liquid was cooled to 30° C., and adjusted to the pH within a range of from 7 to 8 by use of 25% aqueous ammonia. Thus, an emulsion was prepared, and this emulsion was applied to a dry glass plate, and then only the polymer component from the resultant coating was extracted with chloroform. This extract was analyzed by <sup>1</sup>H-NMR measurement, and the vinyl chloride/ethyl acrylate ratio was determined to be 90:10 as the composition of the above-prepared emulsion-1.

##### (Synthesis of Emulsion-2)

Emulsion-2 was prepared in the same manner as the Emulsion-1, except that the amount of vinyl chloride used was changed. The amount is shown in Table 1, together with the elastic modulus of the latex polymer prepared.

TABLE 1

| Latex      | Polymer composition |                     | Elastic modulus (MPa) |
|------------|---------------------|---------------------|-----------------------|
|            | Vinyl chloride unit | Ethyl acrylate unit |                       |
| Emulsion-1 | 90                  | 10                  | 1700                  |
| Emulsion-2 | 70                  | 30                  | 800                   |

## (Preparation of Emulsified Dispersion A)

An emulsified dispersion A was prepared in the following manner. An antioxidant agent (EB-9) was dissolved in a mixture of 42 g of a high-boiling solvent (Solv-5) and 20 ml of ethyl acetate, and the resulting solution was emulsified and dispersed in 250 g of a 20 mass % aqueous gelatin solution containing 1 g of sodium dodecylbenzenesulfonate by means of a high-speed stirring emulsification machine (dissolver). Thereto, water was added to prepare 380 g of an emulsified dispersion A.

Therein, the addition amount of the antioxidant agent (EB-9) was adjusted so that the antioxidant agent would be contained in an amount of 30 mol % in the emulsified dispersion A.

## (Preparation of Heat-Sensitive Transfer Image-Receiving Sheet 101 (Comparative Example))

A sample was prepared by simultaneous multi-layer coating, so as to form a multiple-layer structure, on the support prepared in the foregoing manner, having a subbing layer, a heat insulation layer, and a receptor layer, in increasing order of distance from the support. Compositions and application amounts of the coating solutions used herein are shown below.

Coating solution for subbing layer  
(Composition)

|                                                                                 |                  |
|---------------------------------------------------------------------------------|------------------|
| Latex styrene/butadiene (SR103 (trade name), manufactured by Nippon A & L Inc.) | 93 parts by mass |
| 8.7% Aqueous solution of polyvinyl alcohol (PVA)                                | 57 parts by mass |
| NaOH for adjusting pH to 8                                                      |                  |
| (Coating amount) 21 ml/m <sup>2</sup>                                           |                  |

Coating solution for heat insulation layer  
(Composition)

|                                                                                        |                  |
|----------------------------------------------------------------------------------------|------------------|
| Hollow latex polymer particles (MH5055 (trade name), manufactured by Zeon Corporation) | 38 parts by mass |
| 16% Gelatin aqueous solution                                                           | 26 parts by mass |
| Water                                                                                  | 4 parts by mass  |
| NaOH for adjusting pH to 8                                                             |                  |
| (Coating amount) 45 ml/m <sup>2</sup>                                                  |                  |

Coating solution for receptor layer (1)  
(Composition)

|                                                                                            |                  |
|--------------------------------------------------------------------------------------------|------------------|
| Latex polymer 1 synthesized in the above (the above emulsion-1, solid content 40% by mass) | 50 parts by mass |
| 10% Gelatin aqueous solution                                                               | 10 parts by mass |
| Emulsified dispersion A prepared in the above                                              | 13 parts by mass |
| Microcrystalline wax (EMUSTAR-42X (trade name), manufactured by Nippon Seiro Co., Ltd.)    | 7 parts by mass  |
| Water                                                                                      | 35 parts by mass |
| NaOH for adjusting pH to 8                                                                 |                  |
| (Coating amount) 18 ml/m <sup>2</sup>                                                      |                  |

Immediately before coating, a compound X (cross-linking agent) illustrated below was added to the foregoing receptor layer coating solution. The amount of the compound X added was adjusted to 3 mass % based on the total mass of gelatin in the heat-insulating layer and the receptor layer.

Compound X



## 10 (Preparation of Heat-Sensitive Transfer Image-Receiving Sheet 102 (Comparative Example))

A heat-sensitive transfer image-receiving sheet 102 was prepared in the same manner as the heat-sensitive transfer image-receiving sheet 101, except that the latex polymer 1 (the above emulsion-1) used in the receptor layer was replaced with the latex polymer 2 synthesized (the above emulsion-2) in this example. Incidentally, the latex polymer 2 was added in the same amount as the latex polymer 1 on a solids basis.

## 20 (Preparation of Heat-Sensitive Transfer Image-Receiving Sheet 103 (Comparative Example))

A heat-sensitive transfer image-receiving sheet 103 was prepared in the same manner as the heat-sensitive transfer image-receiving sheet 101, except that the latex polymer 1 used in the receptor layer was replaced with a commercially available latex polymer Z446 (trade name, manufactured by Goo Chemical Co., Ltd.).

## 25 (Preparation of Heat-Sensitive Transfer Image-Receiving Sheet 104 (This Invention))

A heat-sensitive transfer image-receiving sheet 104 was prepared in the same manner as the heat-sensitive transfer image-receiving sheet 101, except that the latex polymer 1 used in the receptor layer was replaced with a mixture of latex polymer 1 and latex polymer 2 (latex polymer 1 latex polymer 2=50:50).

## 30 35 Preparation of Heat-Sensitive Transfer Image-Receiving Sheet 105 (This Invention))

A heat-sensitive transfer image-receiving sheet 105 was prepared in the same manner as the heat-sensitive transfer image-receiving sheet 101, except that the latex polymer 1 used in the receptor layer was replaced with a mixture of latex polymer 1, latex polymer 2 and latex polymer Z446 (trade name, manufactured by Goo Chemical Co., Ltd., elastic modulus: 20 MPa) (latex polymer 1 latex polymer 2: latex polymer Z446=40:40:20).

## 40 45 (Preparation of Heat-Sensitive Transfer Image-Receiving Sheet 106 (This Invention))

A heat-sensitive transfer image-receiving sheet 106 was prepared in the same manner as the heat-sensitive transfer image-receiving sheet 101, except that the latex polymer 1 used in the receptor layer (the coating solution for receptor layer (1) containing latex polymer 1 was coated in an amount of 18 ml/m<sup>2</sup>) was replaced with the coating solution for receptor layer (1) containing latex polymer I (9 ml/m<sup>2</sup>) as an upper layer and a coating solution for receptor layer (2) containing latex polymer 2 (9 ml/m<sup>2</sup>) as a lower layer were multi-layer coated.

## 50 (Preparation of Heat-Sensitive Transfer Image-Receiving Sheet 107 (This Invention))

A heat-sensitive transfer image-receiving sheet 107 was prepared in the same manner as the heat-sensitive transfer image-receiving sheet 101, except that the latex polymer 1 used in the receptor layer (the coating solution for receptor layer (1) containing latex polymer 1 was coated in an amount of 18 ml/m<sup>2</sup>) was replaced with the coating solution for receptor layer (2) containing latex polymer 2 (9 ml/m<sup>2</sup>) as an upper layer and the receptor-layer-coating solution for receptor layer (3) containing polyester-series latex polymer Z446 (9 ml/m<sup>2</sup>) as a lower layer which were multi-layer coated.

In the above, the coating solution for receptor layer (2) and the coating solution for receptor layer (3) were prepared in the same manner as the coating solution for the receptor layer (1), except that the latex polymer 1 was replaced with the same amount (solid basis) of the latex polymer 2 and the latex polymer Z446, respectively.

A list of Heat-sensitive transfer image-receiving sheets 101 to 107 is shown in Table 2 set forth below.

TABLE 2

|                                                                 | Sample No.                      |                                 |                                 |                            |                            |                            |                            |
|-----------------------------------------------------------------|---------------------------------|---------------------------------|---------------------------------|----------------------------|----------------------------|----------------------------|----------------------------|
|                                                                 | 101<br>(Comparative<br>Example) | 102<br>(Comparative<br>Example) | 103<br>(Comparative<br>Example) | 104<br>(This<br>invention) | 105<br>(This<br>invention) | 106<br>(This<br>invention) | 107<br>(This<br>invention) |
| Kind of latex polymer(s)<br>having different elastic<br>modulus | 1                               | 1                               | 1                               | 2                          | 3                          | 2                          | 2                          |
| Composition of receptor<br>layer                                | Polymer 1                       | Polymer 2                       | Z446                            | Polymer 1<br>Polymer 2     | Polymer 1<br>Polymer 2     | Polymer 1<br>Polymer 2     | Z446                       |
| Coating method                                                  | —                               | —                               | —                               | mixture                    | mixture                    | 2 layers                   | 2 layers                   |

## (Image Formation)

The ink sheet and any of the heat-sensitive transfer image-receiving sheets 101 to 107 were each worked so as to become loadable, and a printed output was produced on each combination of the ink sheet and any of the image-receiving sheets, in a high-speed print mode, by use of a sublimation-type thermal transfer printer ASK2000 (trade name, manufactured by FUJIFILM Corporation). More specifically, the black image (black solid image) of the maximum density on the entire face was used as an output image, and the output image was produced in succession on 20 pieces of each image-receiving sheet. Herein, the time interval between ejection of one printed piece and ejection of the next one was 8 seconds.

These evaluation results of sticking and noises caused by processing were ranked as shown below, and the results are shown in Table 3.

## Evaluation Rank

- ◎: Better results than the level for ○ were obtained.  
○: Good results were obtained without any problems.  
Δ: Results obtained showed tendencies to deteriorate, but they were still on an acceptable level.

x: Results obtained had problems, so that they were on a practically unacceptable level.

## (3) Evaluation of White Spot Image Defect

Subsequent to output of gray at a highlight portion, the white spot image defect was evaluated by examining a degree of blur in low sensitivity regions.

## Evaluation Rank

- ◎: Better results than the level for ○ were obtained.  
○: Good results were obtained without any problems.  
Δ: Results obtained showed tendencies to deteriorate, but they were still on an acceptable level.

x: Results obtained had problems, so that they were on a practically unacceptable level.

TABLE 3

| Evaluation<br>of properties | Sample No. (Remarks)            |                                 |                                 |                            |                            |                            |                            |
|-----------------------------|---------------------------------|---------------------------------|---------------------------------|----------------------------|----------------------------|----------------------------|----------------------------|
|                             | 101<br>(Comparative<br>Example) | 102<br>(Comparative<br>Example) | 103<br>(Comparative<br>Example) | 104<br>(This<br>invention) | 105<br>(This<br>invention) | 106<br>(This<br>invention) | 107<br>(This<br>invention) |
|                             | Polymer 1                       | Polymer 2                       | Z446                            | Polymer 1<br>Polymer 2     | Polymer 1<br>Polymer 2     | Polymer 1<br>Polymer 2     | Z446                       |
| Dmax                        | —                               | —                               | —                               | Mixture                    | Mixture                    | 2 layers                   | 2 layers                   |
| Releasing property          | ○                               | X                               | Δ                               | 2.03                       | 2.00                       | 2.04                       | 2.02                       |
| White-spot image<br>defect  | X                               | ◎                               | X                               | ○                          | ○                          | ○                          | Δ                          |

## (Image Evaluation)

## (1) Evaluation of Dmax

The visual density of the black solid image obtained in the above condition was measured by Photographic Densitometer (trade name, manufactured by X-Rite Incorporated).

## (2) Evaluation of Releasing Property (Adhesive Property)

For evaluation of releasing property of the image-receiving sheet from the ink sheet, the black image (black solid image) of the maximum density on the entire face was output, on each image-receiving sheet in accordance with the foregoing method, and the surface of the obtained outputs were observed to evaluate the extent of streaked unevenness (sticking) on the surface thereof. At the same time, noises caused by this processing were caught and their volume was evaluated.

From the results of samples 101 to 107, it is understood that properties of the heat-sensitive transfer image-receiving sheet (i.e., Dmax, releasing property, white spot image defect) remarkably changed depending on how the latex polymers which had different elastic moduli from each other were used. From comparisons among Samples 101 to 105, it is understood that Samples 104 and 105 each of which used the mixture of latex polymers having different elastic moduli from each other exhibited better performance, compared to Samples 101 to 103 each of which used the latex polymer singly. In addition, from comparisons among Samples 104 to 107, it is understood that Samples 106 and 107 which used the latex polymers having different elastic moduli from each other in the two-layer structure exhibited better performance.

From the results of samples 101 to 107, it is understood that properties of the heat-sensitive transfer image-receiving sheet (i.e., Dmax, releasing property, white spot image defect) remarkably changed depending on how the latex polymers which had different elastic moduli from each other were used. From comparisons among Samples 101 to 105, it is understood that Samples 104 and 105 each of which used the mixture of latex polymers having different elastic moduli from each other exhibited better performance, compared to Samples 101 to 103 each of which used the latex polymer singly. In addition, from comparisons among Samples 104 to 107, it is understood that Samples 106 and 107 which used the latex polymers having different elastic moduli from each other in the two-layer structure exhibited better performance.

41

In the case where the two-layer structure is formed, it is preferable to form a two-layer structure using a pair of polymers having a complementary relation, as seen in the samples 106 and 107. Specifically, it is preferably to use a latex polymer that is excellent in releasing property (generally, a latex polymer having a high elastic modulus) for the upper layer of the receptor layer, whereas a latex polymer that is excellent in cushion property (generally, a latex polymer having a low elastic modulus) for the lower layer of the receptor layer. The thus-obtained heat-sensitive transfer image-receiving sheet having two-layer structure shows such effective performances that are hardly achieved by a single use of each latex polymer.

## Example 2

Using the heat-sensitive transfer image-receiving sheets prepared in Example 1, image formation was performed in the same manner as Example 1, except that the printer was changed to a sublimation-type thermal transfer printer CW01 (trade name, manufactured by Citizen). The thus-obtained Samples were evaluated in the same manner as in Example 1. The heat-sensitive transfer image-receiving sheets according to the present invention also exhibited good results as in the case of Example 1.

Having described our invention as related to the present embodiments, it is our intention that the invention not be limited by any of the details of the description, unless otherwise specified, but rather be construed broadly within its spirit and scope as set out in the accompanying claims.

What we claim is:

1. A sublimation-type heat-sensitive transfer image-receiving sheet, comprising:

a support;

at least one receptor layer containing at least two kinds of latex polymers, said latex polymers having different elastic moduli from each other; and

at least one heat-insulation layer containing hollow latex polymer particles and a water-soluble polymer, said at least one heat-insulation layer being provided between the support and the at least one receptor layer,

wherein at least one of the at least two kinds of latex polymers is a copolymer containing repeating units derived from vinyl chloride and units derived from  $\alpha,\beta$ -unsaturated carboxylate or a copolymer containing repeating units derived from vinyl chloride and units derived from vinyl ester.

2. The sublimation-type heat-sensitive transfer image-receiving sheet according to claim 1, wherein, among the latex polymers contained in the receptor layer, an elastic modulus of a latex polymer having the lowest elastic modulus is 1500 MPa or less, and an elastic modulus of a latex polymer having the highest elastic modulus is 1600 MPa or more, but 2200 MPa or less.

3. A sublimation-type heat-sensitive transfer image-receiving sheet, comprising:

a support;

at least one receptor layer containing at least two kinds of latex polymers, said latex polymers having different elastic moduli from each other; and

at least one heat-insulation layer containing hollow latex polymer particles and a water-soluble polymer, said at least one heat-insulation layer being provided between the support and the at least one receptor layer,

wherein at least one of the at least two kinds of latex polymers is a copolymer containing repeating units derived from vinyl chloride and units derived from  $\alpha,\beta$ -

42

unsaturated carboxylate or a copolymer containing repeating units derived from vinyl chloride and units derived from vinyl ester, and

wherein the receptor layer includes an upper layer and a lower layer, and a latex-polymer composition of the upper layer is different from that of the lower layer.

4. The sublimation-type heat-sensitive transfer image-receiving sheet according to claim 3, wherein the upper layer comprises the latex polymer having the highest elastic modulus in a highest proportion; and the lower layer comprises the latex polymer having the lowest elastic modulus in a highest proportion.

5. The sublimation-type heat-sensitive transfer image-receiving sheet according to claim 1, wherein the receptor layer further contains a water-soluble polymer.

6. The sublimation-type heat-sensitive transfer image-receiving sheet according to claim 1, wherein at least one of the at least two kinds of latex polymers is a copolymer containing repeating units derived from vinyl chloride and repeating units derived from  $\alpha,\beta$ -unsaturated carboxylate.

7. A sublimation-type heat-sensitive transfer image-receiving sheet comprising:

a support;

at least one receptor layer containing at least two kinds of latex polymers, said latex polymers having different elastic moduli from each other; and

at least one heat-insulation layer containing hollow latex polymer particles and a water-soluble polymer, said at least one heat-insulation layer being provided between the support and the at least one receptor layer,

wherein at least one of the at least two kinds of latex polymers is a copolymer containing repeating units derived from vinyl chloride and units derived from  $\alpha,\beta$ -unsaturated carboxylate or a copolymer containing repeating units derived from vinyl chloride and units derived from vinyl ester, and

wherein the at least two kinds of latex polymers each comprises repeating units derived from vinyl chloride.

8. The sublimation-type heat-sensitive transfer image-receiving sheet according to claim 3,

wherein the receptor layer includes an upper layer and a lower layer, the lower layer being closest to the heat insulation layer, and the upper layer being a layer which contacts to an ink sheet at the time of image formation, and

wherein the elastic modulus of the latex polymer contained in the lower layer is lower than that of the latex polymer contained in the upper layer.

9. The sublimation-type heat-sensitive transfer image-receiving sheet according to claim 1, wherein glass transition temperature of at least one of the latex polymers is 0°C. to 80°C.

10. The sublimation-type heat-sensitive transfer image-receiving sheet according to claim 3, wherein, among the latex polymers contained in the receptor layer, an elastic modulus of a latex polymer having the lowest elastic modulus is 1500 MPa or less, and an elastic modulus of a latex polymer having the highest elastic modulus is 1600 MPa or more, but 2200 MPa or less.

11. The sublimation-type heat-sensitive transfer image-receiving sheet according to claim 3, wherein the receptor layer further contains a water-soluble polymer.

12. The sublimation-type heat-sensitive transfer image-receiving sheet according to claim 3, wherein the receptor layer and the heat insulation layer are simultaneous applied, in the production process of the heat-sensitive transfer image-receiving sheet.

43

13. The sublimation-type heat-sensitive transfer image-receiving sheet according to claim 3, wherein the receptor layer and the heat insulation layer are applied by simultaneous multilayer coating of using aqueous coating solutions.

14. The sublimation-type heat-sensitive transfer image-receiving sheet according to claim 3, wherein at least one of the at least two kinds of latex polymers is a copolymer containing repeating units derived from vinyl chloride and repeating units derived from  $\alpha,\beta$ -unsaturated carboxylate.

15. A sublimation-type heat-sensitive transfer image-receiving sheet, comprising:

a support;

at least one receptor layer containing at least two kinds of latex polymers, said latex polymers having different elastic moduli from each other; and

at least one heat-insulation layer containing hollow latex polymer particles and a water-soluble polymer, said at least one heat-insulation layer being provided between the support and the at least one receptor layer,

wherein at least one of the at least two kinds of latex polymers is a copolymer containing repeating units derived from vinyl chloride and units derived from  $\alpha,\beta$ -unsaturated carboxylate or a copolymer containing repeating units derived from vinyl chloride and units derived from vinyl ester,

wherein the receptor layer includes an upper layer and a lower layer, and a latex-polymer composition of the upper layer is different from that of the lower layer, and wherein the at least two kinds of latex polymers each comprises repeating units derived from vinyl chloride.

16. The sublimation-type heat-sensitive transfer image-receiving sheet according to claim 3, wherein glass transition temperature of at least one of the latex polymers is 0° C. to 80° C.

17. A sublimation-type heat-sensitive transfer image-receiving sheet, comprising:

a support;

at least one receptor layer containing at least two kinds of latex polymers, said latex polymers having different elastic moduli from each other; and

at least one heat-insulation layer containing hollow latex polymer particles and gelatin, said at least one heat-

5

10

15

20

25

30

35

40

44

insulation layer being provided between the support and the at least one receptor layer,

wherein at least one of the at least two kinds of latex polymers is a copolymer containing repeating units derived from vinyl chloride and units derived from  $\alpha,\beta$ -unsaturated carboxylate or a copolymer containing repeating units derived from vinyl chloride and units derived from vinyl ester, and

wherein, among the latex polymers contained in the receptor layer, an elastic modulus of a latex polymer having the lowest elastic modulus is 1500 MPa or less, and an elastic modulus of a latex polymer having the highest elastic modulus is 1600 MPa or more, but 2200 MPa or less.

18. The sublimation-type heat-sensitive transfer image-receiving sheet according to claim 17, wherein the at least two kinds of latex polymers each comprises repeating units derived from vinyl chloride.

19. The sublimation-type heat-sensitive transfer image-receiving sheet according to claim 7,

wherein the at least two kinds of latex polymers each comprising repeating units derived from vinyl chloride each are a copolymer containing repeating units derived from vinyl chloride and units derived from unsaturated  $\alpha,\beta$ -carboxylate.

20. The sublimation-type heat-sensitive transfer image-receiving sheet according to claim 15,

wherein the at least two kinds of latex polymers each comprising repeating units derived from vinyl chloride each are a copolymer containing repeating units derived from vinyl chloride and units derived from unsaturated  $\alpha,\beta$ -carboxylate.

21. The sublimation-type heat-sensitive transfer image-receiving sheet according to claim 18,

wherein the at least two kinds of latex polymers each comprising repeating units derived from vinyl chloride each are a copolymer containing repeating units derived from vinyl chloride and units derived from unsaturated  $\alpha,\beta$ -carboxylate.

\* \* \* \* \*